



US007579078B2

(12) **United States Patent**  
**Hartmann et al.**

(10) **Patent No.:** **US 7,579,078 B2**  
(45) **Date of Patent:** **Aug. 25, 2009**

(54) **TEMPERATURE REGULATING  
CELLULOSIC FIBERS AND APPLICATIONS  
THEREOF**

(75) Inventors: **Mark H. Hartmann**, Superior, CO (US); **James B. Worley**, Westminster, CO (US); **Matthew North**, Bad Abbach (DE)

(73) Assignee: **Outlast Technologies, Inc.**, Boulder, CO (US)

(\*) Notice: Subject to any disclaimer, the term of this patent is extended or adjusted under 35 U.S.C. 154(b) by 0 days.

(21) Appl. No.: **11/495,156**

(22) Filed: **Jul. 27, 2006**

(65) **Prior Publication Data**

US 2007/0026228 A1 Feb. 1, 2007

**Related U.S. Application Data**

(63) Continuation-in-part of application No. 10/638,290, filed on Aug. 7, 2003, now Pat. No. 7,244,497, which is a continuation-in-part of application No. 10/052,232, filed on Jan. 15, 2002, now Pat. No. 6,855,422, which is a continuation-in-part of application No. 09/960,591, filed on Sep. 21, 2001, now abandoned.

(51) **Int. Cl.**

**D02G 3/00** (2006.01)

**B32B 9/00** (2006.01)

**D04H 1/00** (2006.01)

(52) **U.S. Cl.** ..... **428/373**; 428/374; 428/393; 428/402; 428/402.2; 428/402.21; 428/401; 442/361

(58) **Field of Classification Search** ..... 428/373, 428/374, 393, 402, 402.2, 402.21, 401

See application file for complete search history.

(56) **References Cited**

U.S. PATENT DOCUMENTS

1,902,529 A 3/1933 Stockley et al.  
4,756,958 A 7/1988 Bryant et al.

(Continued)

FOREIGN PATENT DOCUMENTS

AT 384628 B1 5/1987

(Continued)

OTHER PUBLICATIONS

PCT Notification of Transmittal of International Search Report and the Written Opinion of the International Searching Authority, or the Declaration, PCT/US07/73789, Dec. 27, 2007, 3 pages.

(Continued)

*Primary Examiner*—Lynda Salvatore

(74) *Attorney, Agent, or Firm*—Neugeboren O'Dowd PC

(57) **ABSTRACT**

Cellulosic fibers having enhanced reversible thermal properties and applications of such cellulosic fibers are described. In one embodiment, a cellulosic fiber includes a fiber body including a cellulosic material and a set of microcapsules dispersed in the cellulosic material. The set of microcapsules contain a phase change material having a latent heat of at least 40 J/g and a transition temperature in the range of 0° C. to 100° C., and the phase change material provides thermal regulation based on at least one of absorption and release of the latent heat at the transition temperature. The cellulosic fiber can be formed via a solution spinning process, and can be used in various products where thermal regulating properties are desired.

**13 Claims, 5 Drawing Sheets**



## U.S. PATENT DOCUMENTS

4,908,238 A 3/1990 Vigo et al.  
 5,153,066 A \* 10/1992 Tanaka et al. .... 428/373  
 5,993,710 A 11/1999 Weigel et al.  
 6,319,599 B1 11/2001 Buckley  
 6,793,856 B2 \* 9/2004 Hartmann et al. .... 264/141  
 2002/0054964 A1 5/2002 Hartmann  
 2003/0035951 A1 2/2003 Magill et al.  
 2004/0126555 A1 7/2004 Hartmann et al.  
 2004/0241399 A1 \* 12/2004 Marmon et al. .... 428/196  
 2005/0090175 A1 4/2005 Bergholm et al.

## FOREIGN PATENT DOCUMENTS

DE 2164189 A1 8/1972  
 DE 4446491 C2 6/1996  
 DE 3751894 T2 9/1996  
 DE 202004021259 U1 5/2007  
 EP 0311642 B1 9/1996  
 GB 1390939 A1 4/1975  
 GB 2121069 A 5/1983  
 GB 2121069 A1 12/1983  
 GB 2324064 A 10/1998  
 JP 08170224 A 7/1996  
 JP 2000192326 A 7/2000  
 JP 2000192326 A1 7/2000  
 WO 98/46814 A1 10/1998  
 WO 9846814 A1 10/1998  
 WO WO 03027365 A1 4/2003  
 WO WO 2005024102 A1 3/2005

## OTHER PUBLICATIONS

PCT Written Opinion of the International Searching Authority, PCT/US07/73789, Dec. 27, 2007, 5 pages.  
 Request For Ex Parte Reexamination, U.S. Appl. No. 90/010,121 dated Mar. 12, 2008, 32 pages.  
 Claim chart submitted in Re-examination U.S. Appl. No. 90/010,121, filed Mar. 12, 2008, 14 pages.

Falbe and Regitz, Rompp Chemie Lexikon, 9th Edition [1989] p. 102, Georg Thieme Verlag Stuttgart, New York, 4 pages, with English translation.

Falbe and Regitz, Rompp Chemie Lexikon, 9th Edition [1989], p. 616, 4 pages, with English translation.

Falbe and Regitz, Rompp Chemie Lexikon, 9th edition [1991], p. 3216, Georg Thieme Verlag Stuttgart, New York, 4 pages, with English translation.

Corrected Request For Ex Parte Reexamination, U.S. Appl. No. 90/010,121 dated Apr. 17, 2008, including corrected claim chart, 51 pages.

Order Granting Request for ex parte reexamination, U.S. Appl. No. 90/101,121 dated Jun. 25, 2008, 20 pages.

Lorenz and Kollegen, "Response to Request for Nullification of German Utility Model No. DE 20 2004 021 259", Jul. 9, 2008, Published in: Germany.

Exxonmobil Corporation, "Mobilcer 46—Emulsion de cera", Unknown, Published in: Argentina.

Zounek Plate Schweitzer, "Request for Nullification of German Utility Model No. DE 20 2004 021 259 U1", Dec. 4, 2007, Published in: Germany.

Falbe and Regitz, "Rompp Chemie Lexicon", 1989, p. 102, 103, 616, 624, 3185, 3216, 9th Ed., Publisher: Georg Thieme Verlag, Published in: Stuttgart/New York.

German Patent Office, "Office Action Letter in Nullification Action for DE 20 2004 021 259", Sep. 15, 2008, p. 4, Publisher: German Patent Office, Published in: Germany.

European Patent Office, "Supplementary European Search Report in Application No. EP 04 75 7345", Oct. 10, 2008, p. 2, Published in: The Hague.

Tao, Xiaoming, "Smart Fibres, Fabrics and Clothing", 2001, pp. 34-57, Publisher: Woodhead Publishing, XP002492889, Published in: US.

Summary English Translation of German Patent Office, "Office Action Letter in Nullification Action for DE 20 2004 021 259", Sep. 15, 2008, p. 1.

German Patent Office, Written Argumentation in German Nullification Action re German Utility Model No. 20 2004 021 259, Mar. 18, 2009, 18 pages.

\* cited by examiner



FIG. 1



FIG. 2



FIG. 3



FIG. 4



FIG. 5





FIG. 7

## 1

**TEMPERATURE REGULATING  
CELLULOSIC FIBERS AND APPLICATIONS  
THEREOF**

**CROSS-REFERENCE TO RELATED  
APPLICATIONS**

This application is a continuation-in-part of the patent application of Hartmann et al., entitled "Cellulosic Fibers Having Enhanced Reversible Thermal Properties and Methods of Forming Thereof," U.S. application Ser. No. 10/638,290, filed on Aug. 7, 2003 now U.S. Pat. No. 7,244,497, which is a continuation-in-part of the patent application of Magill et al., entitled "Multi-component Fibers Having Enhanced Reversible Thermal Properties and Methods of Manufacturing Thereof," U.S. application Ser. No. 10/052,232, filed on Jan. 15, 2002 now U.S. Pat. No. 6,855,422, which is a continuation-in-part of the patent application of Magill et al., entitled "Multi-component Fibers Having Enhanced Reversible Thermal Properties," U.S. application Ser. No. 09/960,591, filed on Sep. 21, 2001 now abandoned, the disclosures of which are incorporated herein by reference in their entireties.

**FIELD OF THE INVENTION**

The invention relates to fibers having enhanced reversible thermal properties. For example, cellulosic fibers having enhanced reversible thermal properties and applications of such cellulosic fibers are described.

**BACKGROUND OF THE INVENTION**

Many fibers are formed from naturally occurring polymers. Various processing operations can be required to convert these polymers into fibers. In some instances, the resulting fibers can be referred to as regenerated fibers.

An important class of regenerated fibers includes fibers formed from cellulose. Cellulose is a significant component of plant matter, such as, for example, leaves, wood, bark, and cotton. Conventionally, a solution spinning process is used to form fibers from cellulose. A wet solution spinning process is conventionally used to form rayon fibers and lyocell fibers, while a dry solution spinning process is conventionally used to form acetate fibers. Rayon fibers and lyocell fibers often include cellulose having the same or similar chemical structure as naturally occurring cellulose. However, cellulose included in these fibers often has a shorter molecular chain length relative to naturally occurring cellulose. For example, rayon fibers often include cellulose in which substituents have replaced not more than about 15 percent of hydrogens of hydroxyl groups in the cellulose. Examples of rayon fibers include viscose rayon fibers and cuprammonium rayon fibers. Acetate fibers often include a chemically modified form of cellulose in which various hydroxyl groups are replaced by acetyl groups.

Fibers formed from cellulose find numerous applications. For example, these fibers can be used to form knitted or woven fabrics, which can be incorporated in products such as apparel or footwear. Fabrics formed from these fibers are generally perceived as comfort fabrics due to their ability to take up moisture and their low retention of body heat. These properties make the fabrics desirable in warm weather by allowing a wearer to feel cooler. However, these same properties can make the fabrics undesirable in cold weather. In cold and damp weather, the fabrics can be particularly undesirable due to rapid removal of body heat when the fabrics are wet. As another example, fibers formed from cellulose can be

## 2

used to form non-woven fabrics, which can be incorporated in products such as personal hygiene products or medical products. Non-woven fabrics formed from these fibers are generally perceived as desirable due to their ability to take up moisture. However, for similar reasons as discussed above, the non-woven fabrics generally fail to provide a desirable level of comfort, particularly under changing environmental conditions.

It is against this background that a need arose to develop the 10 cellulosic fibers described herein.

**SUMMARY OF THE INVENTION**

In one innovative aspect, the invention relates to a cellulosic fiber. In one embodiment, the cellulosic fiber includes a fiber body including a cellulosic material and a set of micro-capsules dispersed in the cellulosic material. The set of micro-capsules contain a phase change material having a latent heat of at least 40 J/g and a transition temperature in the range of 0° C. to 100° C., and the phase change material provides thermal regulation based on at least one of absorption and release of the latent heat at the transition temperature.

In another innovative aspect, the invention relates to a fabric. In one embodiment, the fabric includes a set of cellulosic fibers blended together. The set of cellulosic fibers include a cellulosic fiber having enhanced reversible thermal properties and including a fiber body including an elongated member. The elongated member includes a cellulosic material and a temperature regulating material dispersed within the cellulosic material, and the temperature regulating material includes a phase change material having a transition temperature in the range of 0° C. to 50° C.

Other aspects and embodiments of the invention are also contemplated. For example, other aspects of the invention relate to a method of forming a cellulosic fiber, a method of forming a fabric, a method of providing thermal regulation using a cellulosic fiber, and a method of providing thermal regulation using a fabric. The foregoing summary and the following detailed description are not meant to restrict the invention to any particular embodiment but are merely meant to describe some embodiments of the invention.

**BRIEF DESCRIPTION OF THE DRAWINGS**

For a better understanding of the nature and objects of various embodiments of the invention, reference should be made to the following detailed description taken in conjunction with the accompanying drawings.

FIG. 1 illustrates a three-dimensional view of a cellulosic fiber according to an embodiment of the invention.

FIG. 2 illustrates a three-dimensional view of another cellulosic fiber according to an embodiment of the invention.

FIG. 3 illustrates cross-sectional views of various cellulosic fibers according to an embodiment of the invention.

FIG. 4 illustrates cross-sectional views of additional cellulosic fibers according to an embodiment of the invention.

FIG. 5 illustrates a three-dimensional view of a cellulosic fiber having a core-sheath configuration, according to an embodiment of the invention.

FIG. 6 illustrates a three-dimensional view of another cellulosic fiber having a core-sheath configuration, according to an embodiment of the invention.

FIG. 7 illustrates a three-dimensional view of a cellulosic fiber having an island-in-sea configuration, according to an embodiment of the invention.

## DETAILED DESCRIPTION

Embodiments of the invention relate to fibers having enhanced reversible thermal properties and applications of such fibers. In particular, various embodiments of the invention relate to cellulosic fibers including phase change materials. Cellulosic fibers in accordance with various embodiments of the invention have the ability to absorb and release thermal energy under different environmental conditions. In addition, the cellulosic fibers can exhibit improved processability (e.g., during formation of the cellulosic fibers or a product made therefrom), lower costs (e.g., during formation of the cellulosic fibers or a product made therefrom), improved mechanical properties, improved containment of a phase change material within the cellulosic fibers, and higher loading levels of the phase change material.

Cellulosic fibers in accordance with various embodiments of the invention can provide an improved level of comfort when incorporated in products such as, for example, apparel, footwear, personal hygiene products, and medical products. In particular, the cellulosic fibers can provide such improved level of comfort under different environmental conditions. The use of phase change materials allows the cellulosic fibers to exhibit "dynamic" heat retention rather than "static" heat retention. Heat retention typically refers to the ability of a material to retain heat (e.g., body heat). A low level of heat retention is often desired in warm weather, while a high level of heat retention is often desired in cold weather. Unlike conventional fibers formed from cellulose, cellulosic fibers in accordance with various embodiments of the invention can exhibit different levels of heat retention under changing environmental conditions. For example, the cellulosic fibers can exhibit a low level of heat retention in warm weather and a high level of heat retention in cold weather, thus maintaining a desired level of comfort under changing weather conditions.

In conjunction with exhibiting "dynamic" heat retention, cellulosic fibers in accordance with various embodiments of the invention can exhibit a high level of moisture absorbency. Moisture absorbency typically refers to the ability of a material to absorb or take up moisture. In some instances, moisture absorbency of a material can be expressed as a percentage weight gain resulting from absorbed moisture relative to a moisture-free weight of the material under a particular environmental condition (e.g., 21° C. and 65 percent relative humidity). Cellulosic fibers in accordance with various embodiments of the invention can exhibit moisture absorbency of at least 5 percent, such as from about 6 percent to about 15 percent, from about 6 percent to about 13 percent, or from about 11 percent to about 13 percent. A high level of moisture absorbency can serve to reduce the amount of skin moisture, such as due to perspiration. In the case of personal hygiene products, this high level of moisture absorbency can also serve to draw moisture away from the skin and to trap the moisture, thereby reducing or preventing skin irritation or rashes. In addition, moisture absorbed by cellulosic fibers can enhance the heat conductivity of the cellulosic fibers. Thus, for example, when incorporated in apparel or footwear, the cellulosic fibers can serve to reduce the amount of skin moisture as well as lower skin temperature, thereby providing a higher level of comfort in warm weather. The use of phase change materials in the cellulosic fibers further enhances the level of comfort by absorbing or releasing thermal energy to maintain a comfortable skin temperature.

In addition, cellulosic fibers in accordance with various embodiments of the invention can exhibit other desirable properties. For example, when incorporated in non-woven fabrics, the cellulosic fibers can have one or more of the

following properties: (1) a sink time that is from about 2 seconds to about 60 seconds, such as from about 3 seconds to about 20 seconds or from about 4 seconds to about 10 seconds; (2) a tensile strength that is from about 13 cN/tex to about 40 cN/tex, such as from about 16 cN/tex to about 30 cN/tex or from about 18 cN/tex to about 25 cN/tex; (3) an elongation at break that is from about 10 percent to about 40 percent, such as from about 14 percent to about 30 percent or from about 17 percent to about 22 percent; and (4) a shrinkage in boiling water that is from about 0 percent to about 6 percent, such as from about 0 percent to about 4 percent or from about 0 percent to about 3 percent.

A cellulosic fiber according to some embodiments of the invention can include a set of elongated members. As used herein, the term "set" refers to a collection of one or more objects. In some instances, the cellulosic fiber can include a fiber body formed of the set of elongated members. The fiber body is typically elongated and can have a length that is several times (e.g., 100 times or more) greater than its diameter. In some instances, a staple length of the fiber body can be from about 0.3 mm to about 100 mm, such as from about 4 mm to about 75 mm or from about 20 mm to about 50 mm. The fiber body can have any of various regular or irregular cross-sectional shapes, such as circular, C-shaped, indented, flower petal-shaped, multi-limbed or multi-lobal, octagonal, oval, pentagonal, rectangular, ring-shaped, serrated, square-shaped, star-shaped, trapezoidal, triangular, wedge-shaped, and so forth. Various elongated members of the set of elongated members can be coupled (e.g., bonded, combined, joined, or united) to one another to form a unitary fiber body.

According to some embodiments of the invention, a cellulosic fiber can be formed of at least one elongated member that includes a temperature regulating material. Typically, the temperature regulating material includes one or more phase change materials to provide the cellulosic fiber with enhanced reversible thermal properties. For certain applications, a cellulosic fiber can be formed of various elongated members that can include the same cellulosic material or different cellulosic materials, and at least one elongated member has a temperature regulating material dispersed therein. It is contemplated that one or more elongated members can be formed from various other types of polymeric materials. Typically, the temperature regulating material is substantially uniformly dispersed within at least one elongated member. However, depending upon the particular characteristics desired for the cellulosic fiber, the dispersion of the temperature regulating material can be varied within one or more elongated members. Various elongated members can include the same temperature regulating material or different temperature regulating materials.

Depending upon the particular application, a set of elongated members forming a cellulosic fiber can be arranged in one of various configurations. For example, the set of elongated members can include various elongated members arranged in a core-sheath configuration or an island-in-sea configuration. The elongated members can be arranged in other configurations, such as, for example, a matrix or checkerboard configuration, a segmented-pie configuration, a side-by-side configuration, a striped configuration, and so forth. In some instances, the elongated members can be arranged in a bundle form in which the elongated members are generally parallel with respect to one another. One or more elongated members can extend through at least a portion of a length of a fiber body, and, in some instances, the elongated members can be longitudinally co-extensive. For example, the cellulosic fiber can include an inner member that substantially extends through the length of the cellulosic fiber and includes

a temperature regulating material. The extent to which the inner member extends through the cellulosic fiber can depend upon, for example, desired thermal regulating properties for the cellulosic fiber. In addition, other factors (e.g., desired mechanical properties or method of forming the cellulosic fiber) can play a role in determining this extent. Thus, in some instances, the inner member can extend through from about a half up to the entire length of the cellulosic fiber to provide desired thermal regulating properties. An outer member can surround the inner member and form an exterior of the cellulosic fiber.

According to some embodiments of the invention, a cellulosic fiber can be from about 0.1 to about 1,000 denier or from about 0.1 to about 100 denier. Typically, a cellulosic fiber according to some embodiments of the invention is from about 0.5 to about 15 denier, such as from about 1 to about 15 denier or from about 0.5 to about 10 denier. As one of ordinary skill in the art will understand, a denier typically refers to a measure of weight per unit length of a fiber and represents the number of grams per 9,000 meters of the fiber. According to other embodiments of the invention, a cellulosic fiber can be from about 0.1 decitex to about 60 decitex, such as from about 1 decitex to about 5 decitex or from about 1.3 decitex to about 3.6 decitex. As one of ordinary skill in the art will understand, a decitex typically refers to another measure of weight per unit length of a fiber and represents the number of grams per 10,000 meters of the fiber.

If desired, a cellulosic fiber according to some embodiments of the invention can be further processed to form one or more smaller denier fibers. For example, various elongated members forming the cellulosic fiber can be split apart or fibrillated to form two or more smaller denier fibers, and each smaller denier fiber can include one or more elongated members. It is contemplated that one or more elongated members (or a portion or portions thereof) forming the cellulosic fiber can be mechanically separated, pneumatically separated, dissolved, melted, or otherwise removed to yield one or more smaller denier fibers. Typically, at least one resulting smaller denier fiber includes a temperature regulating material to provide desired thermal regulating properties.

Depending upon the particular application, a cellulosic fiber can also include one or more additives. An additive can be dispersed within one or more elongated members forming the cellulosic fiber. Examples of additives include water, surfactants, dispersants, anti-foam agents (e.g., silicone containing compounds and fluorine containing compounds), antioxidants (e.g., hindered phenols and phosphites), thermal stabilizers (e.g., phosphites, organophosphorous compounds, metal salts of organic carboxylic acids, and phenolic compounds), light or UV stabilizers (e.g., hydroxy benzoates, hindered hydroxy benzoates, and hindered amines), microwave absorbing additives (e.g., multifunctional primary alcohols, glycerine, and carbon), reinforcing fibers (e.g., carbon fibers, aramid fibers, and glass fibers), conductive fibers or particles (e.g., graphite or activated carbon fibers or particles), lubricants, process aids (e.g., metal salts of fatty acids, fatty acid esters, fatty acid ethers, fatty acid amides, sulfonamides, polysiloxanes, organophosphorous compounds, silicon containing compounds, fluorine containing compounds, and phenolic polyethers), fire retardants (e.g., halogenated compounds, phosphorous compounds, organophosphates, organobromides, alumina trihydrate, melamine derivatives, magnesium hydroxide, antimony compounds, antimony oxide, and boron compounds), anti-blocking additives (e.g., silica, talc, zeolites, metal carbonates, and organic polymers), anti-fogging additives (e.g., non-ionic surfactants, glycerol esters, polyglycerol esters, sorbitan esters and their ethoxy-

lates, nonyl phenyl ethoxylates, and alcohol ethoxylates), anti-static additives (e.g., non-ionic such as fatty acid esters, ethoxylated alkylamines, diethanolamides, and ethoxylated alcohol; anionics such as alkylsulfonates and alkylphosphates; cationics such as metal salts of chlorides, methosulfates or nitrates, and quaternary ammonium compounds; and amphoteric such as alkylbetaines), anti-microbials (e.g., arsenic compounds, sulfur, copper compounds, isothiazolins phthalamides, carbamates, silver base inorganic agents, silver zinc zeolites, silver copper zeolites, silver zeolites, metal oxides, and silicates), crosslinkers or controlled degradation agents (e.g., peroxides, azo compounds, silanes, isocyanates, and epoxies), colorants, pigments, dyes, dulling agents (e.g., titanium oxide or  $TiO_2$ ), fluorescent whitening agents or optical brighteners (e.g., bis-benzoxazoles, phenylcoumarins, and bis-(styryl)biphenyls), fillers (e.g., natural minerals and metals such as oxides, hydroxides, carbonates, sulfates, and silicates; talc; clay; wollastonite; graphite; carbon black; carbon fibers; glass fibers and beads; ceramic fibers and beads; metal fibers and beads; flours; and fibers of natural or synthetic origin such as fibers of wood, starch, or cellulose flours), coupling agents (e.g., silanes, titanates, zirconates, fatty acid salts, anhydrides, epoxies, and unsaturated polymeric acids), reinforcement agents, crystallization or nucleation agents (e.g., any material which increases or improves the crystallinity of a polymer, such as to improve rate or kinetics of crystal growth, number of crystals grown, or types of crystals grown), and so forth.

According to some embodiments of the invention, certain additives, treatments, finishes, binders, or coatings can be applied to, or incorporated within, a cellulosic fiber (or a resulting fabric) to impart improved properties such as stain resistance, water repellency, softer feel, and moisture management properties. For example, improved moisture absorbency can be achieved by applying or incorporating hydrophilic or polar materials, such as materials including acids, acid salts, hydroxyl groups (e.g., natural hydroxyl-containing materials), ethers, esters, amines, amine salts, amides, imines, urethanes, sulfones, sulfides, polyquaternary compounds, glycols, polyethylene glycols, natural saccharides, cellulose, sugars, proteins, polymers or high molecular weight molecules that include one or more functional groups, and materials that include two or more functional groups that are the same or different. These materials can be added during a fiber manufacturing process, applied as a finish to a cellulosic fiber, or applied during a fabric manufacturing or finishing process. Advantageously, certain of these materials, such as glycols, polyethylene glycols, and ethers, can also serve as phase change materials, as further discussed below. Other examples of treatments and coatings include Epic (available from Nextec Applications Inc., Vista, Calif.), Intera (available from Intera Technologies, Inc., Chattanooga, Tenn.), Zonyl Fabric Protectors (available from DuPont Inc., Wilmington, Del.), Scotchgard (available from 3M Co., Maplewood, Minn.), and so forth.

The foregoing discussion provides a general overview of some embodiments of the invention. Attention now turns to FIG. 1, which illustrates a three-dimensional view of a cellulosic fiber 1 according to an embodiment of the invention.

As illustrated in FIG. 1, the cellulosic fiber 1 is a mono-component fiber that includes a single elongated member 2. The elongated member 2 is generally cylindrical and includes a cellulosic material 3 and a temperature regulating material 4 dispersed within the cellulosic material 3. In the illustrated embodiment, the temperature regulating material 4 can include various microcapsules containing a phase change material, and the microcapsules can be substantially uni-

formly dispersed throughout the elongated member 2. While it may be desirable to have the microcapsules uniformly dispersed within the elongated member 2, such configuration is not necessary in all applications. The cellulosic fiber 1 can include various percentages by weight of the cellulosic material 3 and the temperature regulating material 4 to provide desired thermal regulating properties, mechanical properties (e.g., ductility, tensile strength, and hardness), and moisture absorbency.

FIG. 2 illustrates a three-dimensional view of another cellulosic fiber 5 according to an embodiment of the invention. As discussed for the cellulosic fiber 1, the cellulosic fiber 5 is a mono-component fiber that includes a single elongated member 6. The elongated member 6 is generally cylindrical and includes a cellulosic material 7 and a temperature regulating material 8 dispersed within the cellulosic material 7. In the illustrated embodiment, the temperature regulating material 8 can include a phase change material in a raw form (e.g., the phase change material is non-encapsulated, i.e., not micro- or macroencapsulated), and the phase change material can be substantially uniformly dispersed throughout the elongated member 6. While it may be desirable to have the phase change material uniformly dispersed within the elongated member 6, such configuration is not necessary in all applications. As illustrated in FIG. 2, the phase change material can form distinct domains that are dispersed within the elongated member 6. The cellulosic fiber 5 can include various percentages by weight of the cellulosic material 7 and the temperature regulating material 8 to provide desired thermal regulating properties, mechanical properties, and moisture absorbency.

FIG. 3 illustrates cross-sectional views of various cellulosic fibers 90, 93, 96, and 99, according to an embodiment of the invention. As illustrated in FIG. 3, each cellulosic fiber (e.g., the cellulosic fiber 90) is a mono-component fiber having a cross-section that is multi-limbed or multi-lobial. Such multi-limbed shape can provide a greater "free" volume within a resulting fabric, which, in turn, can provide a higher level of moisture absorbency. Such multi-limbed shape can also provide a greater surface area for enhanced and quicker moisture absorbency, along with channels for movement and wicking of moisture away from the skin.

As illustrated in FIG. 3, the cellulosic fiber 90 has a cross-section that is generally X-shaped, and includes a cellulosic material 91 and a temperature regulating material 92 dispersed within the cellulosic material 91. The cellulosic fiber 93 has a cross-section that is generally Y-shaped, and includes a cellulosic material 94 and a temperature regulating material 95 dispersed within the cellulosic material 94. As illustrated in FIG. 3, the cellulosic fiber 96 has a cross-section that is generally T-shaped, and includes a cellulosic material 97 and a temperature regulating material 98 dispersed within the cellulosic material 97. And, the cellulosic fiber 99 has a cross-section that is generally H-shaped, and includes a cellulosic material 100 and a temperature regulating material 101 dispersed within the cellulosic material 100.

If desired, a length-to-width ratio of limbs included in the cellulosic fibers 90, 93, 96, and 99 can be adjusted so as to provide a desired balance between mechanical properties and moisture absorbency. For example, in the case of the cellulosic fiber 90, a ratio of L to W of each limb (e.g., a limb 102) can be from about 1 to about 15, such as from about 2 to about 10, from about 2 to about 7, or from about 3 to about 5.

Turning next to FIG. 4, cross-sectional views of various cellulosic fibers 12, 13, 14, 21, 22, 23, 24, 26, 27, 28, 29, and 34 are illustrated, according to an embodiment of the invention. As illustrated in FIG. 4, each cellulosic fiber (e.g., the

cellulosic fiber 21) is a multi-component fiber that includes various distinct cross-sectional regions. These cross-sectional regions correspond to various elongated members (e.g., elongated members 39 and 40) that form each cellulosic fiber.

5 In the illustrated embodiment, each cellulosic fiber includes a first set of elongated members (shown shaded in FIG. 4) and a second set of elongated members (shown unshaded in FIG. 4). Here, the first set of elongated members can be formed from a cellulosic material that has a temperature 10 regulating material dispersed therein. The second set of elongated members can be formed from the same cellulosic material or another cellulosic material having somewhat different properties. In general, various elongated members of the first set of elongated members can be formed from the 15 same cellulosic material or different cellulosic materials. Similarly, various elongated members of the second set of elongated members can be formed from the same cellulosic material or different cellulosic materials. It is contemplated that one or more elongated members can be formed from various other types of polymeric materials.

For certain applications, a temperature regulating material 20 can be dispersed within a second set of elongated members. Different temperature regulating materials can be dispersed within the same elongated member or different elongated members. For example, a first temperature regulating material 25 can be dispersed within a first set of elongated members, and a second temperature regulating material having somewhat different properties can be dispersed within a second set of elongated members. It is contemplated that one or more elongated members 30 can be formed from a temperature regulating material that need not be dispersed within a cellulosic material or other polymeric material. For example, the temperature regulating material can include a polymeric phase change material that provides enhanced reversible thermal properties and that can be used to form a first set of elongated members. In this case, it may be desirable, but not required, that a second set of elongated members adequately surround the first set of elongated members to reduce or prevent loss or leakage of the temperature regulating material. Various elongated 35 members 40 can be formed from the same polymeric phase change material or different polymeric phase change materials.

In the illustrated embodiment, each cellulosic fiber can 45 include various percentages by weight of a first set of elongated members that include a temperature regulating material relative to a second set of elongated members. For example, when thermal regulating properties of a cellulosic fiber are a controlling consideration, a larger proportion of the cellulosic fiber can include a first set of elongated members that include 50 a temperature regulating material. On the other hand, when mechanical properties and moisture absorbency of the cellulosic fiber are a controlling consideration, a larger proportion of the cellulosic fiber can include a second set of elongated members that need not include the temperature regulating material. Alternatively, when balancing thermal regulating 55 properties and other properties of the cellulosic fiber, it can be desirable that the second set of elongated members include the same or a different temperature regulating material.

For example, a cellulosic fiber in the illustrated embodiment 60 can include from about 1 percent to about 99 percent by weight of a first set of elongated members. Typically, the cellulosic fiber includes from about 10 percent to about 90 percent by weight of the first set of elongated members. As an example, a cellulosic fiber can include 90 percent by weight of a first elongated member and 10 percent by weight of a second elongated member. For this example, the first elongated member can include 60 percent by weight of a tempera-

ture regulating material, such that the cellulosic fiber includes 54 percent by weight of the temperature regulating material. As another example, the cellulosic fiber can include up to about 50 percent by weight of the first elongated member, which in turn can include up to about 50 percent by weight of the temperature regulating material. Such weight percentages provide the cellulosic fiber with up to about 25 percent by weight of the temperature regulating material and provide effective thermal regulating properties, mechanical properties, and moisture absorbency for the cellulosic fiber. It is contemplated that a percentage by weight of an elongated member relative to a total weight of a cellulosic fiber can be varied, for example, by adjusting a cross-sectional area of the elongated member or by adjusting the extent to which the elongated member extends through a length of the cellulosic fiber.

Referring to FIG. 4, left-hand column 10 illustrates three cellulosic fibers 12, 13, and 14. The cellulosic fiber 12 includes various elongated members arranged in a segmented-pie configuration. In the illustrated embodiment, a first set of elongated members 15, 15', 15", 15'', and 15''' and a second set of elongated members 16, 16', 16", 16'', and 16''' are arranged in an alternating fashion and have cross-sections that are wedge-shaped. In general, the elongated members can have cross-sectional shapes and areas that are the same or different. While the cellulosic fiber 12 is illustrated with ten elongated members, it is contemplated that, in general, two or more elongated members can be arranged in a segmented-pie configuration, and at least one of the elongated members typically will include a temperature regulating material.

The cellulosic fiber 13 includes various elongated members arranged in an island-in-sea configuration. In the illustrated embodiment, a first set of elongated members (e.g., elongated members 35, 35', 35", and 35'''') are positioned within and surrounded by a second elongated member 36, thereby forming "islands" within a "sea." Such configuration can serve to provide a more uniform distribution of a temperature regulating material within the cellulosic fiber 13. In the illustrated embodiment, the first set of elongated members have cross-sections that are trapezoidal. In general, the first set of elongated members can have cross-sectional shapes and areas that are the same or different. While the cellulosic fiber 13 is illustrated with seventeen elongated members positioned within and surrounded by the second elongated member 36, it is contemplated that, in general, one or more elongated members can be positioned within and surrounded by the second elongated member 36.

The cellulosic fiber 14 includes various elongated members arranged in a striped configuration. In the illustrated embodiment, a first set of elongated members 37, 37', 37", 37'', and 37''' and a second set of elongated members 38, 38', 38'', and 38''' are arranged in an alternating fashion and are shaped as longitudinal slices of the cellulosic fiber 14. In general, the elongated members can have cross-sectional shapes and areas that are the same or different. The cellulosic fiber 14 can be a self-crimping or self-texturing fiber and can impart loft, bulk, insulation, stretch, or other like properties. While the cellulosic fiber 14 is illustrated with nine elongated members, it is contemplated that, in general, two or more elongated members can be arranged in a striped configuration, and at least one of the elongated members typically will include a temperature regulating material.

For the cellulosic fibers 12 and 14, one or more elongated members (e.g., the elongated member 15) of a first set of elongated members can be partially surrounded by one or more adjacent elongated members (e.g., the elongated members 16 and 16'''). When an elongated member including a

phase change material is not completely surrounded, it may be desirable, but not required, that a containment structure (e.g., microcapsules) is used to contain the phase change material dispersed within the elongated member. In some instances, the cellulosic fibers 12, 13, and 14 can be further processed to form one or more smaller denier fibers. Thus, for example, the elongated members forming the cellulosic fiber 12 can be split apart, or one or more elongated members (or a portion or portions thereof) can be dissolved, melted, or otherwise removed. A resulting smaller denier fiber can include, for example, the elongated members 15 and 16 coupled to one another.

Middle column 20 of FIG. 4 illustrates four cellulosic fibers 21, 22, 23, and 24. In particular, the cellulosic fibers 21, 22, 23, and 24 each includes various elongated members arranged in a core-sheath configuration.

The cellulosic fiber 21 includes a first elongated member 39 positioned within and surrounded by a second elongated member 40. More particularly, the first elongated member 39 is formed as a core member that includes a temperature regulating material. This core member is concentrically positioned within and completely surrounded by the second elongated member 40 that is formed as a sheath member. In the illustrated embodiment, the cellulosic fiber 21 can include about 25 percent by weight of the core member and about 75 percent by weight of the sheath member.

As discussed for the cellulosic fiber 21, the cellulosic fiber 22 includes a first elongated member 41 positioned within and surrounded by a second elongated member 42. The first elongated member 41 is formed as a core member that includes a temperature regulating material. This core member is concentrically positioned within and completely surrounded by the second elongated member 42 that is formed as a sheath member. In the illustrated embodiment, the cellulosic fiber 22 can include about 50 percent by weight of the core member and about 50 percent by weight of the sheath member.

The cellulosic fiber 23 includes a first elongated member 43 positioned within and surrounded by a second elongated member 44. Here, the first elongated member 43 is formed as a core member that is eccentrically positioned within the second elongated member 44 that is formed as a sheath member. The cellulosic fiber 23 can include various percentages by weight of the core member and the sheath member to provide desired thermal regulating properties, mechanical properties, and moisture absorbency.

As illustrated in FIG. 4, the cellulosic fiber 24 includes a first elongated member 45 positioned within and surrounded by a second elongated member 46. In the illustrated embodiment, the first elongated member 45 is formed as a core member that has a tri-lobal cross-sectional shape. This core member is concentrically positioned within the second elongated member 46 that is formed as a sheath member. The cellulosic fiber 24 can include various percentages by weight of the core member and the sheath member to provide desired thermal regulating properties, mechanical properties, and moisture absorbency.

It is contemplated that, in general, a core member can have any of various regular or irregular cross-sectional shapes, such as, for example, circular, indented, flower petal-shaped, multi-lobal, octagonal, oval, pentagonal, rectangular, serrated, square-shaped, trapezoidal, triangular, wedge-shaped, and so forth. While the cellulosic fibers 21, 22, 23, and 24 are each illustrated with one core member positioned within and surrounded by a sheath member, it is contemplated that two or more core members can be positioned within and surrounded by a sheath member (e.g., in a manner similar to that illus-

## 11

trated for the cellulosic fiber 13). These two or more core members can have cross-sectional shapes and areas that are the same or different. It is also contemplated that a cellulosic fiber can include three or more elongated members arranged in a core-sheath configuration, such that the elongated members are shaped as concentric or eccentric longitudinal slices of the cellulosic fiber. Thus, for example, the cellulosic fiber can include a core member positioned within and surrounded by a sheath member, which, in turn, is positioned within and surrounded by another sheath member.

Right-hand column 30 of FIG. 4 illustrates five cellulosic fibers 26, 27, 28, 29, and 34. In particular, the cellulosic fibers 26, 27, 28, 29, and 34 each includes various elongated members arranged in a side-by-side configuration.

The cellulosic fiber 26 includes a first elongated member 47 positioned adjacent to and partially surrounded by a second elongated member 48. In the illustrated embodiment, the elongated members 47 and 48 have half-circular cross-sectional shapes. Here, the cellulosic fiber 26 can include about 50 percent by weight of the first elongated member 47 and about 50 percent by weight of the second elongated member 48. The elongated members 47 and 48 also can be characterized as being arranged in a segmented-pie or a striped configuration.

As discussed for the cellulosic fiber 26, the cellulosic fiber 27 includes a first elongated member 49 positioned adjacent to and partially surrounded by a second elongated member 50. In the illustrated embodiment, the cellulosic fiber 27 can include about 20 percent by weight of the first elongated member 49 and about 80 percent by weight of the second elongated member 50. The elongated members 49 and 50 also can be characterized as being arranged in a core-sheath configuration, such that the first elongated member 49 is eccentrically positioned with respect to and partially surrounded by the second elongated member 50.

The cellulosic fibers 28 and 29 are examples of mixed-viscosity fibers. The cellulosic fibers 28 and 29 each includes a first elongated member 51 or 53 that has a temperature regulating material dispersed therein and is positioned adjacent to and partially surrounded by a second elongated member 52 or 54.

A mixed-viscosity fiber can be considered to be a self-crimping or self-texturing fiber, such that the fiber's crimping or texturing can impart loft, bulk, insulation, stretch, or other like properties. Typically, a mixed-viscosity fiber includes various elongated members that are formed from different polymeric materials. The different polymeric materials used to form the mixed-viscosity fiber can include polymers with different viscosities, chemical structures, or molecular weights. When the mixed-viscosity fiber is drawn, uneven stresses can be created between various elongated members, and the mixed-viscosity fiber can crimp or bend. In some instances, the different polymeric materials used to form the mixed-viscosity fiber can include polymers having different degrees of crystallinity. For example, a first polymeric material used to form a first elongated member can have a lower degree of crystallinity than a second polymeric material used to form a second elongated member. When the mixed-viscosity fiber is drawn, the first and second polymeric materials can undergo different degrees of crystallization to "lock" an orientation and strength into the mixed-viscosity fiber. A sufficient degree of crystallization can be desired to prevent or reduce reorientation of the mixed-viscosity fiber during subsequent processing (e.g., heat treatment).

For example, for the cellulosic fiber 28, the first elongated member 51 can be formed from a first cellulosic material, and the second elongated member 52 can be formed from a second cellulosic material having somewhat different properties.

## 12

It is contemplated that the first elongated member 51 and the second elongated member 52 can be formed from the same cellulosic material, and a temperature regulating material can be dispersed within the first elongated member 51 to impart self-crimping or self-texturing properties to the cellulosic fiber 28. It is also contemplated that the first elongated member 51 can be formed from a polymeric phase change material, and the second elongated member 52 can be formed from a cellulosic material having somewhat different properties.

10 The cellulosic fibers 28 and 29 can include various percentages by weight of the first elongated members 51 and 53 and the second elongated members 52 and 54 to provide desired thermal regulating properties, mechanical properties, moisture absorbency, and self-crimping or self-texturing properties.

15 The cellulosic fiber 34 is an example of an ABA fiber. As illustrated in FIG. 4, the cellulosic fiber 34 includes a first elongated member 55 positioned between and partially surrounded by a second set of elongated members 56 and 56'. In the illustrated embodiment, the first elongated member 55 is formed from a cellulosic material that has a temperature regulating material dispersed therein. Here, the second set of elongated members 56 and 56' can be formed from the same cellulosic material or another cellulosic material having somewhat different properties. In general, the elongated members 55, 56, and 56' can have cross-sectional shapes and areas that are the same or different. The elongated members 55, 56, and 56' also can be characterized as being arranged in a striped configuration.

20 Attention next turns to FIG. 5, which illustrates a three-dimensional view of a cellulosic fiber 59 having a core-sheath configuration, according to an embodiment of the invention. The cellulosic fiber 59 includes an elongated and generally cylindrical core member 57 positioned within and surrounded by an elongated and annular-shaped sheath member 58. In the illustrated embodiment, the core member 57 substantially extends through a length of the cellulosic fiber 59 and is completely surrounded or encased by the sheath member 58, which forms an exterior of the cellulosic fiber 59. In general, the core member 57 can be concentrically or eccentrically positioned within the sheath member 58.

25 As illustrated in FIG. 5, the core member 57 includes a temperature regulating material 61 dispersed therein. In the illustrated embodiment, the temperature regulating material 61 can include various microcapsules containing a phase change material, and the microcapsules can be substantially uniformly dispersed throughout the core member 57. While it may be desirable to have the microcapsules uniformly dispersed within the core member 57, such configuration is not necessary in all applications. The core member 57 and the sheath member 58 can be formed from the same cellulosic material or different cellulosic materials. It is contemplated that either, or both, of the core member 57 and the sheath member 58 can be formed from various other types of polymeric materials. The cellulosic fiber 59 can include various percentages by weight of the core member 57 and the sheath member 58 to provide desired thermal regulating properties, mechanical properties, and moisture absorbency.

30 FIG. 6 illustrates a three-dimensional view of another cellulosic fiber 60 having a core-sheath configuration, according to an embodiment of the invention. As discussed for the cellulosic fiber 59, the cellulosic fiber 60 includes an elongated and generally cylindrical core member 63 substantially extending through a length of the cellulosic fiber 60. The core member 63 is positioned within and completely surrounded or encased by an elongated and annular-shaped sheath mem-

ber 64, which forms an exterior of the cellulosic fiber 60. In general, the core member 63 can be concentrically or eccentrically positioned within the sheath member 64.

As illustrated in FIG. 6, the core member 63 includes a temperature regulating material 62 dispersed therein. Here, the temperature regulating material 62 can include a phase change material in a raw form, and the phase change material can be substantially uniformly dispersed throughout the core member 63. While it may be desirable to have the phase change material uniformly dispersed within the core member 63, such configuration is not necessary in all applications. In the illustrated embodiment, the phase change material can form distinct domains that are dispersed within the core member 63. By surrounding the core member 63, the sheath member 64 can serve to enclose the phase change material within the core member 63. Accordingly, the sheath member 64 can reduce or prevent loss or leakage of the phase change material during fiber formation or during end use. The core member 63 and the sheath member 64 can be formed from the same cellulosic material or different cellulosic materials. It is contemplated that either, or both, of the core member 63 and the sheath member 64 can be formed from various other types of polymeric materials. Thus, for example, it is contemplated that the core member 63 can be formed from a polymeric phase change material that need not be dispersed in a cellulosic material. The cellulosic fiber 60 can include various percentages by weight of the core member 63 and the sheath member 64 to provide desired thermal regulating properties, mechanical properties, and moisture absorbency.

Referring to FIG. 7, a three-dimensional view of a cellulosic fiber 70 having an island-in-sea configuration is illustrated, according to an embodiment of the invention. The cellulosic fiber 70 includes a set of elongated and generally cylindrical island members 72, 73, 74, and 75 positioned within and surrounded by an elongated sea member 71. In the illustrated embodiment, the island members 72, 73, 74, and 75 substantially extend through a length of the cellulosic fiber 70 and are completely surrounded or encased by the sea member 71, which forms an exterior of the cellulosic fiber 70. While four island members are illustrated, it is contemplated that the cellulosic fiber 70 can include more or less islands members depending upon the particular application of the cellulosic fiber 70.

One or more temperature regulating materials can be dispersed within the island members 72, 73, 74, and 75. As illustrated in FIG. 7, the cellulosic fiber 70 includes two different temperature regulating materials 80 and 81. The island members 72 and 75 include the temperature regulating material 80, while the island members 73 and 74 include the temperature regulating material 81. In the illustrated embodiment, the temperature regulating materials 80 and 81 can include different phase change materials in a raw form, and the phase change materials can form distinct domains that are dispersed within respective island members. By surrounding the island members 72, 73, 74, and 75, the sea member 71 can serve to enclose the phase change materials within the island members 72, 73, 74, and 75.

In the illustrated embodiment, the sea member 71 is formed of a sea cellulosic material 82, and the island members 72, 73, 74, and 75 are formed of island cellulosic materials 76, 77, 78, and 79, respectively. The sea cellulosic material 82 and the island cellulosic materials 76, 77, 78, and 79 can be the same or can differ from one another in some fashion. It is contemplated that one or more of the sea member 71 and the island members 72, 73, 74, and 75 can be formed from various other types of polymeric materials. Thus, for example, it is contemplated that one or more of the island members 72, 73, 74, and

75 can be formed from a polymeric phase change material that need not be dispersed in a cellulosic material. The cellulosic fiber 70 can include various percentages by weight of the sea member 71 and the island members 72, 73, 74, and 75 to provide desired thermal regulating properties, mechanical properties, and moisture absorbency.

As discussed previously, a cellulosic fiber according to some embodiments of the invention can include one or more temperature regulating materials. A temperature regulating material typically includes one or more phase change materials. In general, a phase change material can be any substance (or any mixture of substances) that has the capability of absorbing or releasing thermal energy to regulate, reduce, or eliminate heat flow within a temperature stabilizing range. The temperature stabilizing range can include a particular transition temperature or a particular range of transition temperatures. A phase change material used in conjunction with various embodiments of the invention typically is capable of inhibiting a flow of thermal energy during a time when the phase change material is absorbing or releasing heat, typically as the phase change material undergoes a transition between two states (e.g., liquid and solid states, liquid and gaseous states, solid and gaseous states, or two solid states). This action is typically transient. In some instances, a phase change material can effectively inhibit a flow of thermal energy until a latent heat of the phase change material is absorbed or released during a heating or cooling process. Thermal energy can be stored or removed from a phase change material, and the phase change material typically can be effectively recharged by a source of heat or cold. By selecting an appropriate phase change material, a cellulosic fiber can be designed for use in any of various products.

For certain applications, a phase change material can be a solid/solid phase change material. A solid/solid phase change material is a type of phase change material that undergoes a transition between two solid states (e.g., a crystalline or mesocrystalline phase transformation) and hence typically does not become a liquid during use.

A phase change material can include a mixture of two or more substances. By selecting two or more different substances and forming a mixture, a temperature stabilizing range can be adjusted over a wide range for any particular application of a cellulosic fiber. In some instances, a mixture of two or more different substances can exhibit two or more distinct transition temperatures or a single modified transition temperature when incorporated in a cellulosic fiber.

Phase change materials that can be used in conjunction with various embodiments of the invention include various organic and inorganic substances. Examples of phase change materials include hydrocarbons (e.g., straight-chain alkanes or paraffinic hydrocarbons, branched-chain alkanes, unsaturated hydrocarbons, halogenated hydrocarbons, and alicyclic hydrocarbons), hydrated salts (e.g., calcium chloride hexahydrate, calcium bromide hexahydrate, magnesium nitrate hexahydrate, lithium nitrate trihydrate, potassium fluoride tetrahydrate, ammonium alum, magnesium chloride hexahydrate, sodium carbonate decahydrate, disodium phosphate dodecahydrate, sodium sulfate decahydrate, and sodium acetate trihydrate), waxes, oils, water, fatty acids, fatty acid esters, dibasic acids, dibasic esters, 1-halides, primary alcohols, secondary alcohols, tertiary alcohols, aromatic compounds, clathrates, semi-clathrates, gas clathrates, anhydrides (e.g., stearic anhydride), ethylene carbonate, polyhydric alcohols (e.g., 2,2-dimethyl-1,3-propanediol, 2-hydroxymethyl-2-methyl-1,3-propanediol, ethylene glycol, polyethylene glycol, pentaerythritol, dipentaerythritol, pentaglycerine, tetramethylol ethane, neopentyl glycol, tet-

ramethylol propane, 2-amino-2-methyl-1,3-propanediol, monoaminopentaerythritol, diaminopentaerythritol, and tris (hydroxymethyl)acetic acid), polymers (e.g., polyethylene, polyethylene glycol, polyethylene oxide, polypropylene, polypropylene glycol, polytetramethylene glycol, polypropylene malonate, polyneopentyl glycol sebacate, polypentane glutarate, polyvinyl myristate, polyvinyl stearate, polyvinyl laurate, polyhexadecyl methacrylate, polyoctadecyl methacrylate, polyesters produced by polycondensation of glycals (or their derivatives) with diacids (or their derivatives), and copolymers, such as polyacrylate or poly(meth) acrylate with alkyl hydrocarbon side chain or with polyethylene glycol side chain and copolymers including polyethylene, polyethylene glycol, polyethylene oxide, polypropylene, polypropylene glycol, or polytetramethylene glycol), metals, and mixtures thereof.

The selection of a phase change material is typically dependent upon a transition temperature or a particular application of a cellulosic fiber that includes the phase change material. A transition temperature of a phase change material typically correlates with a desired temperature or a desired range of temperatures that can be maintained by the phase change material. For example, a phase change material having a transition temperature near room temperature or normal body temperature can be desirable for clothing applications. In particular, cellulosic fibers including such phase change material can be incorporated into apparel or footwear to maintain a comfortable skin temperature for a user. A phase change material having a transition temperature near room temperature or normal body temperature can also be desirable for other applications, such as those related to personal hygiene products or medical products. In some instances, a phase change material can have a transition temperature in the range of about  $-5^{\circ}\text{C}$ . to about  $125^{\circ}\text{C}$ ., such as from about  $0^{\circ}\text{C}$ . to about  $100^{\circ}\text{C}$ ., from about  $0^{\circ}\text{C}$ . to about  $50^{\circ}\text{C}$ ., from about  $15^{\circ}\text{C}$ . to about  $45^{\circ}\text{C}$ ., from about  $22^{\circ}\text{C}$ . to about  $40^{\circ}\text{C}$ ., or from about  $22^{\circ}\text{C}$ . to about  $28^{\circ}\text{C}$ .

The selection of a phase change material can also be dependent upon a latent heat of the phase change material. A latent heat of a phase change material typically correlates with its ability to regulate heat transfer. In some instances, a phase change material can have a latent heat that is at least about 40 J/g, such as at least about 50 J/g, at least about 60 J/g, at least about 70 J/g, at least about 80 J/g, at least about 90 J/g, or at least about 100 J/g. Thus, for example, the phase change material can have a latent heat from about 40 J/g to about 400 J/g, such as from about 60 J/g to about 400 J/g, from about 80 J/g to about 400 J/g, or from about 100 J/g to about 400 J/g.

Particularly useful phase change materials include paraffinic hydrocarbons having from 10 to 44 carbon atoms (i.e.,  $\text{C}_{10}\text{-C}_{44}$  paraffinic hydrocarbons). Table 1 sets forth a list of  $\text{C}_{13}\text{-C}_{28}$  paraffinic hydrocarbons that can be used as phase change materials in the cellulosic fibers described herein. The number of carbon atoms of a paraffinic hydrocarbon typically correlates with its melting point. For example, n-Octacosane, which includes 28 straight-chain carbon atoms per molecule, has a melting point of about  $61.4^{\circ}\text{C}$ . By comparison, n-Tridecane, which includes 13 straight-chain carbon atoms per molecule, has a melting point of about  $-5.5^{\circ}\text{C}$ . n-Octadecane, which includes 18 straight-chain carbon atoms per molecule and has a melting point of about  $28.2^{\circ}\text{C}$ ., can be particularly desirable for clothing applications.

TABLE 1

| Paraffinic Hydrocarbon | No. of Carbon Atoms | Melting Point ( $^{\circ}\text{C}$ .) |
|------------------------|---------------------|---------------------------------------|
| n-Octacosane           | 28                  | 61.4                                  |
| n-Heptacosane          | 27                  | 59.0                                  |
| n-Hexacosane           | 26                  | 56.4                                  |
| n-Pentacosane          | 25                  | 53.7                                  |
| n-Tetracosane          | 24                  | 50.9                                  |
| n-Tricosane            | 23                  | 47.6                                  |
| n-Docosane             | 22                  | 44.4                                  |
| n-Heneicosane          | 21                  | 40.5                                  |
| n-Eicosane             | 20                  | 36.8                                  |
| n-Nonadecane           | 19                  | 32.1                                  |
| n-Octadecane           | 18                  | 28.2                                  |
| n-Heptadecane          | 17                  | 22.0                                  |
| n-Hexadecane           | 16                  | 18.2                                  |
| n-Pentadecane          | 15                  | 10.0                                  |
| n-Tetradecane          | 14                  | 5.9                                   |
| n-Tridecane            | 13                  | -5.5                                  |

Other useful phase change materials include polymeric phase change materials having transition temperatures suitable for a desired application of the resulting cellulosic fibers. Thus, for clothing and other applications, a polymeric phase change material can have a transition temperature in the range of about  $0^{\circ}\text{C}$ . to about  $50^{\circ}\text{C}$ ., such as from about  $22^{\circ}\text{C}$ . to about  $40^{\circ}\text{C}$ .

A polymeric phase change material can include a polymer (or a mixture of polymers) having any of various chain structures and including one or more types of monomer units. In particular, a polymeric phase change material can include a linear polymer, a branched polymer (e.g., a star-branched polymer, a comb-branched polymer, or a dendritic-branched polymer), or a mixture thereof. For certain applications, a polymeric phase change material desirably includes a linear polymer or a polymer with a small amount of branching to allow for a greater density and a greater degree of ordered molecular packing and crystallization. Such greater degree of ordered molecular packing and crystallization can lead to a larger latent heat and a narrower temperature stabilizing range (e.g., a well-defined transition temperature). A polymeric phase change material can include a homopolymer, a copolymer (e.g., a terpolymer, a statistical copolymer, a random copolymer, an alternating copolymer, a periodic copolymer, a block copolymer, a radial copolymer, or a graft copolymer), or a mixture thereof. Properties of one or more types of monomer units forming a polymeric phase change material can affect a transition temperature of the polymeric phase change material. Accordingly, the selection of the monomer units can be dependent upon a desired transition temperature or a desired application of cellulosic fibers that include the polymeric phase change material. As one of ordinary skill in the art will understand, the reactivity and functionality of a polymer can be altered by addition or replacement of one or more functional groups, such as, for example, amines, amides, carboxyls, hydroxyls, esters, ethers, epoxides, anhydrides, isocyanates, silanes, ketones, aldehydes, and so forth. Also, a polymeric phase change material can include a polymer capable of crosslinking, entanglement, or hydrogen bonding in order to increase toughness or resistance to heat, moisture, or chemicals.

As one of ordinary skill in the art will understand, some polymers can be provided in various forms having different molecular weights, since a molecular weight of a polymer can be determined by processing conditions used for forming the polymer. Accordingly, a polymeric phase change material can

include a polymer (or a mixture of polymers) having a particular molecular weight or a particular range of molecular weights. As used herein, the term "molecular weight" can refer to a number average molecular weight or a weight average molecular weight of a polymer (or a mixture of polymers).

For certain applications, a polymeric phase change material can be desirable as a result of having a higher molecular weight, larger molecular size, and higher viscosity relative to non-polymeric phase change materials such as, for example, paraffinic hydrocarbons. As a result of such properties, a polymeric phase change material can exhibit a lesser tendency to leak from a cellulosic fiber during fiber formation or during end use. For some embodiments of the invention, a polymeric phase change material can include polymers having a number average molecular weight in the range of about 400 to about 5,000,000, such as, for example, from about 2,000 to about 5,000,000, from about 8,000 to about 100,000, or from about 8,000 to about 15,000. As one of ordinary skill in the art will understand, a higher molecular weight for a polymer is typically associated with a lower acid number for the polymer. When incorporated within a cellulosic fiber having a core-sheath or island-in-sea configuration, a higher molecular weight or higher viscosity can serve to prevent a polymeric phase change material from flowing through a sheath member or a sea member forming an exterior of the cellulosic fiber. In addition to providing thermal regulating properties, a polymeric phase change material can provide improved mechanical properties when incorporated in cellulosic fibers in accordance with various embodiments of the invention. In some instances, a polymeric phase change material having a desired transition temperature can be mixed with a cellulosic material or other polymeric material to form an elongated member. In other instances, a polymeric phase change material can provide adequate mechanical properties, such that it can be used to form an elongated member without requiring a cellulosic material or other polymeric material. Such configuration can allow for a higher loading level of the polymeric phase change material and improved thermal regulating properties.

For example, polyethylene glycols can be used as phase change materials in some embodiments of the invention. The number average molecular weight of a polyethylene glycol

typically correlates with its melting point. For example, polyethylene glycols having a number average molecular weight in the range of about 570 to about 630 (e.g., Carbowax<sup>TM</sup> 600, available from The Dow Chemical Company, Midland, Mich.) typically have a melting point in the range of about 20° C. to about 25° C., making them desirable for clothing applications. Other polyethylene glycols that can be useful at other temperature stabilizing ranges include polyethylene glycols having a number average molecular weight of about 400 and a melting point in the range of about 4° C. to about 8° C., polyethylene glycols having a number average molecular weight in the range of about 1,000 to about 1,500 and a melting point in the range of about 42° C. to about 48° C., and polyethylene glycols having a number average molecular weight of about 6,000 and a melting point in the range of about 56° C. to about 63° C. (e.g., Carbowax<sup>TM</sup> 400, 1500, and 6000, available from The Dow Chemical Company, Midland, Mich.).

Additional useful phase change materials include polymeric phase change materials based on polyethylene glycols that are endcapped with fatty acids. For example, polyethylene glycol fatty acid diesters having a melting point in the range of about 22° C. to about 35° C. can be formed from polyethylene glycols having a number average molecular weight in the range of about 400 to about 600 that are endcapped with stearic acid or lauric acid. Further useful phase change materials include polymeric phase change materials based on tetramethylene glycol. For example, polytetramethylene glycols having a number average molecular weight in the range of about 1,000 to about 1,800 (e.g., Terathane<sup>®</sup> 1000 and 1800, available from DuPont Inc., Wilmington, Del.) typically have a melting point in the range of about 19° C. to about 36° C. Polyethylene oxides having a melting point in the range of about 60° C. to about 65° C. also can be used as phase change materials in some embodiments of the invention.

For certain applications, polymeric phase change materials can include homopolymers having a melting point in the range of about 0° C. to about 50° C. that can be formed using conventional polymerization processes. Table 2 sets forth melting points of various homopolymers that can be formed from different types of monomer units.

TABLE 2

| Class of Monomer Unit                     | Homopolymer                                                                                     | Melting Point of Homopolymer (° C.) |
|-------------------------------------------|-------------------------------------------------------------------------------------------------|-------------------------------------|
| Acrylates, Methacrylates, and Acrylamides | Polyoctadecyl methacrylate                                                                      | 36                                  |
|                                           | Polyhexadecyl methacrylate                                                                      | 22                                  |
|                                           | Poly-N-tetradecyl polyacrylamide                                                                | 18                                  |
|                                           | Poly-N-tetradecyl polyacrylamide-1,1 dihydroperfluoro                                           | 32-35                               |
| Alkanes and Alkenes                       | Poly-1-decene                                                                                   | 34-40                               |
|                                           | Poly-1-heptene                                                                                  | 17                                  |
|                                           | cis-polyoctenamer (Vestenamer <sup>®</sup> 6213, available from Degussa AG, Frankfurt, Germany) | 38                                  |
|                                           | Poly-1-octene                                                                                   | 5-10                                |
|                                           | Poly-1-nonene                                                                                   | 19-22                               |
|                                           | trans-polypentemer                                                                              | 23-34                               |
|                                           | Poly-1-undecene                                                                                 | 36                                  |
|                                           | cis-polyisoprene                                                                                | 28-36                               |
|                                           | syndiotactic 1,2-poly(1,3-pentadiene)                                                           | 10                                  |
|                                           | 1-methyl-polydodecamethylene                                                                    | 30                                  |

TABLE 2-continued

| Class of Monomer Unit                    | Homopolymer                                                                                                          | Melting Point of Homopolymer (° C.) |
|------------------------------------------|----------------------------------------------------------------------------------------------------------------------|-------------------------------------|
| Ethers                                   | Polymethyleneoxytetramethylene oxide<br>(Poly-1,3-dioxepane)                                                         | 30                                  |
|                                          | Polyhexamethyleneoxymethylene oxide                                                                                  | 38                                  |
|                                          | Polyoxacyclobutane (POX)                                                                                             | 34-36                               |
|                                          | n-octadecyl polyacetaldehyde                                                                                         | 18                                  |
|                                          | Polytetramethylene glycol 1000<br>(Terathane ® polyTHF 1000,<br>available from DuPont Inc.,<br>Wilmington, Delaware) | 25-33                               |
|                                          | Polytetramethylene glycol 1400<br>(Terathane ® polyTHF 1400,<br>available from DuPont Inc.,<br>Wilmington, Delaware) | 27-35                               |
|                                          | Polytetramethylene glycol 1800<br>(Terathane ® polyTHF 1800,<br>available from DuPont Inc.,<br>Wilmington, Delaware) | 27-38                               |
|                                          | Polytetramethylene glycol 2000<br>(Terathane ® polyTHF 2000,<br>available from DuPont Inc.,<br>Wilmington, Delaware) | 28-40                               |
|                                          | Polydodecyl vinyl ether                                                                                              | 30                                  |
|                                          | Polyvinyl laurate                                                                                                    | 16                                  |
| Sulfur Containing Compounds              | Polyvinyl myristate                                                                                                  | 28                                  |
|                                          | 3,3-dimethyl-polytrimethylene sulfide                                                                                | 19                                  |
|                                          | Polymethylene sulfide                                                                                                | 35                                  |
|                                          | Polytetramethylene disulfide                                                                                         | 39-44                               |
| Silicon Containing Compounds             | Polysulfur trioxide                                                                                                  | 32                                  |
|                                          | 1-methyl-trimethylene-poly-sulfonyldivalerate                                                                        | 35                                  |
|                                          | beta-2-polydiethyl siloxane                                                                                          | 17                                  |
|                                          | Nonamethylene-poly-disiloxanylene dipropionamide-diethyl, dimethyl (Si)                                              | 10                                  |
|                                          | Nonamethylene-poly-disiloxanylene dipropionamide-tetraethyl (Si)                                                     | 10                                  |
|                                          | Poly(methyl hexadecyl siloxane                                                                                       | 35                                  |
|                                          | Poly-(hexamethylene)cyclopropylene dicarboxamide-cis-N,N'-dibutyl                                                    | 20                                  |
|                                          | Poly-(hexamethylene)cyclopropylene dicarboxamide-cis-N,N'-diethyl                                                    | 5                                   |
|                                          | Poly-(hexamethylene)cyclopropylene dicarboxamide-cis-N,N'-diisopropyl                                                | 20                                  |
|                                          | Poly-(hexamethylene)cyclopropylene dicarboxamide-cis-N,N'-dimethyl                                                   | 30                                  |
| Amides and Nitrogen Containing Compounds | Poly(pentamethylene adipamide-2,2,3,3,4,4 hexafluoro (diamine)-cis-N,N'-dibutyl                                      | 15                                  |
|                                          | Poly(pentamethylene adipamide-2,2,3,3,4,4 hexafluoro (diamine)-cis-N,N'-diethyl                                      | 20                                  |
|                                          | Poly(pentamethylene adipamide-2,2,3,3,4,4 hexafluoro (diamine)-cis-N,N'-diisopropyl                                  | 35                                  |
|                                          | Poly(pentamethylene adipamide-2,2,3,3,4,4 hexafluoro (diamine)-cis-N,N'-dimethyl                                     | 30                                  |
|                                          | Poly-(4,4'-methylene diphenylene sebacamide)-N,N'-diethyl                                                            | 32                                  |
|                                          | Poly(pentamethylene (hexamethylene disulfonyl)-dicaproamide                                                          | 25                                  |
|                                          | Poly-[ethylene 4,4'-oxydimethylene-di-2-(1,3-dioxolane)-caprylate]                                                   | 19                                  |
|                                          | Poly(pentamethylene adipate-2,2,3,3,4,4 hexa fluoro (4-methyl-(R+)-7-polyhydroxyenanthic acid)                       | 34                                  |
|                                          | Poly-[4-hydroxy tetramethylene-2-(1,3-dioxolane) caprylic acid] (cis or trans)                                       | 36                                  |
|                                          |                                                                                                                      | 23                                  |
|                                          |                                                                                                                      |                                     |
|                                          |                                                                                                                      |                                     |
|                                          |                                                                                                                      |                                     |

TABLE 2-continued

| Class of Monomer Unit | Homopolymer                                      | Melting Point of Homopolymer (° C.) |
|-----------------------|--------------------------------------------------|-------------------------------------|
|                       | Polypentamethylene 2,2'-dibenzoate               | 13                                  |
|                       | Polytetramethylene 2,2'-dibenzoate               | 36                                  |
|                       | Poly-1-methyl-trimethylene 2,2'-dibenzoate       | 38                                  |
|                       | Polycaprolactone glycol (Molecular weight = 830) | 35-45                               |

Polymeric phase change materials can include polyesters having a melting point in the range of about 0° C. to about 40° C. that can be formed by, for example, polycondensation of glycols (or their derivatives) with diacids (or their derivatives). Table 3 sets forth melting points of various polyesters that can be formed from different combinations of glycols and diacids.

TABLE 3

| Glycol                        | Diacid                       | Melting Point of Polyester (° C.) |
|-------------------------------|------------------------------|-----------------------------------|
| Ethylene glycol               | Carbonic                     | 39                                |
| Ethylene glycol               | Pimelic                      | 25                                |
| Ethylene glycol               | Diglycolic                   | 17-20                             |
| Ethylene glycol               | Thiodivaleric                | 25-28                             |
| 1,2-Propylene glycol          | Diglycolic                   | 17                                |
| Propylene glycol              | Malonic                      | 33                                |
| Propylene glycol              | Glutaric                     | 35-39                             |
| Propylene glycol              | Diglycolic                   | 29-32                             |
| Propylene glycol              | Pimelic                      | 37                                |
| 1,3-butanediol                | Sulphenyl divaleric          | 32                                |
| 1,3-butanediol                | Diphenic                     | 36                                |
| 1,3-butanediol                | Diphenyl methane-m,m'-diacid | 38                                |
| 1,3-butanediol                | trans-H,H-terephthalic acid  | 18                                |
| Butanediol                    | Glutaric                     | 36-38                             |
| Butanediol                    | Pimelic                      | 38-41                             |
| Butanediol                    | Azelaic                      | 37-39                             |
| Butanediol                    | Thiodivaleric                | 37                                |
| Butanediol                    | Phthalic                     | 17                                |
| Butanediol                    | Diphenic                     | 34                                |
| Neopentyl glycol              | Adipic                       | 37                                |
| Neopentyl glycol              | Suberic                      | 17                                |
| Neopentyl glycol              | Sebacic                      | 26                                |
| Pantanediol                   | Succinic                     | 32                                |
| Pantanediol                   | Glutaric                     | 22                                |
| Pantanediol                   | Adipic                       | 36                                |
| Pantanediol                   | Pimelic                      | 39                                |
| Pantanediol                   | para-phenyl diacetic acid    | 33                                |
| Pantanediol                   | Diglycolic                   | 33                                |
| Hexanediol                    | Glutaric                     | 28-34                             |
| Hexanediol                    | 4-Octenedioate               | 20                                |
| Heptanediol                   | Oxalic                       | 31                                |
| Octanediol                    | 4-Octenedioate               | 39                                |
| Nonanediol                    | meta-phenylene diglycolic    | 35                                |
| Decanediol                    | Malonic                      | 29-34                             |
| Decanediol                    | Isophthalic                  | 34-36                             |
| Decanediol                    | meso-tartaric                | 33                                |
| Diethylene glycol             | Oxalic                       | 10                                |
| Diethylene glycol             | Suberic                      | 28-35                             |
| Diethylene glycol             | Sebacic                      | 36-44                             |
| Diethylene glycol             | Phthalic                     | 11                                |
| Diethylene glycol             | trans-H,H-terephthalic acid  | 25                                |
| Triethylene glycol            | Sebacic                      | 28                                |
| Triethylene glycol            | Sulphonyl divaleric          | 24                                |
| Triethylene glycol            | Phthalic                     | 10                                |
| Triethylene glycol            | Diphenic                     | 38                                |
| para-dihydroxy-methyl benzene | Malonic                      | 36                                |
| meta-dihydroxy-methyl benzene | Sebacic                      | 27                                |

TABLE 3-continued

| Glycol                        | Diacid     | Melting Point of Polyester (° C.) |
|-------------------------------|------------|-----------------------------------|
| meta-dihydroxy-methyl benzene | Diglycolic | 35                                |

In some instances, a polymeric phase change material having a desired transition temperature can be formed by reacting a phase change material (e.g., a phase change material discussed above) with a polymer (or a mixture of polymers). Thus, for example, n-octadecylic acid (i.e., stearic acid) can be reacted or esterified with polyvinyl alcohol to yield polyvinyl stearate, or dodecanoic acid (i.e., lauric acid) can be reacted or esterified with polyvinyl alcohol to yield polyvinyl laurate. Various combinations of phase change materials (e.g., phase change materials with one or more functional groups such as amine, carboxyl, hydroxyl, epoxy, silane, sulfuric, and so forth) and polymers can be reacted to yield polymeric phase change materials having desired transition temperatures.

Polymeric phase change materials having desired transition temperatures can be formed from various types of monomer units. For example, similar to polyoctadecyl methacrylate, a polymeric phase change material can be formed by polymerizing octadecyl methacrylate, which can be formed by esterification of octadecyl alcohol with methacrylic acid. Also, polymeric phase change materials can be formed by polymerizing a polymer (or a mixture of polymers). For example, poly-(polyethylene glycol)methacrylate, poly-(polyethylene glycol) acrylate, poly-(polytetramethylene glycol)methacrylate, and poly-(polytetramethylene glycol) acrylate can be formed by polymerizing polyethylene glycol methacrylate, polyethylene glycol acrylate, polytetramethylene glycol methacrylate, and polytetramethylene glycol acrylate, respectively. In this example, the monomer units can be formed by esterification of polyethylene glycol (or polytetramethylene glycol) with methacrylic acid (or acrylic acid). It is contemplated that polyglycols can be esterified with allyl alcohol or trans-esterified with vinyl acetate to form polyglycol vinyl ethers, which in turn can be polymerized to form poly-(polyglycol)vinyl ethers. In a similar manner, it is contemplated that polymeric phase change materials can be formed from homologues of polyglycols, such as, for example, ester or ether endcapped polyethylene glycols and polytetramethylene glycols.

According to some embodiments of the invention, a temperature regulating material can include a phase change material in a raw form. During formation of a cellulosic fiber, a phase change material in a raw form can be provided as a solid in any of various forms (e.g., bulk form, powders, pellets,

granules, flakes, and so forth) or as a liquid in any of various forms (e.g., molten form, dissolved in a solvent, and so forth).

According to other embodiments of the invention, a temperature regulating material can include a containment structure that encapsulates, contains, surrounds, absorbs, or reacts with a phase change material. A containment structure can facilitate handling of a phase change material while also offering a degree of protection to the phase change material during formation of a cellulosic fiber or a product made therefrom (e.g., protection from solvents, high temperatures, or shear forces). Moreover, a containment structure can serve to reduce or prevent leakage of a phase change material from a cellulosic fiber during end use. According to some embodiments of the invention, use of a containment structure can be desirable, but not required, when an elongated member having a phase change material dispersed therein is not completely surrounded by another elongated member. Furthermore, it has been discovered that use of a containment structure along with a phase change material can provide various other benefits, such as: (1) providing comparable or superior properties (e.g., in terms of moisture absorbency) relative to a standard cellulosic fiber; (2) allowing for a lower density cellulosic fiber so as to provide a resulting product at lower overall weight; and (3) serving as a less expensive dulling agent that can be used in place of, or in conjunction with, a standard dulling agent (e.g.,  $TiO_2$ ). Without wishing to be bound by a particular theory, it is believed that certain of these benefits result from the relatively low density of certain containment structures as well as the formation of voids within a resulting cellulosic fiber.

For example, a temperature regulating material can include various microcapsules that contain a phase change material, and the microcapsules can be uniformly, or non-uniformly, dispersed within one or more elongated members forming a cellulosic fiber. Microcapsules can be formed as shells enclosing a phase change material, and can include individual microcapsules formed in various regular or irregular shapes (e.g., spherical, spheroidal, ellipsoidal, and so forth) and sizes. The microcapsules can have the same shape or different shapes, and can have the same size or different sizes. As used herein, the term "size" refers to a largest dimension of an object. Thus, for example, a size of a spheroid can refer to a major axis of the spheroid, while a size of a sphere can refer to a diameter of the sphere. In some instances, the microcapsules can be substantially spheroidal or spherical, and can have sizes ranging from about 0.01 to about 4,000 microns, such as from about 0.1 to about 1,000 microns, from about 0.1 to about 500 microns, from about 0.1 to about 100 microns, from about 0.1 to about 20 microns, from about 0.3 to about 5 microns, or from about 0.5 to about 3 microns. For certain implementations, it can be desirable that a substantial fraction, such as at least about 50 percent, at least about 60 percent, at least about 70 percent, at least about 80 percent, or up to about 100 percent, of the microcapsules have sizes within a specified range, such as less than about 12 microns, from about 0.1 to about 12 microns, or from about 0.1 to about 10 microns. It can also be desirable that the microcapsules are monodisperse with respect to either of, or both, their shapes and sizes. As used herein, the term "monodisperse" refers to being substantially uniform with respect to a set of properties. Thus, for example, a set of microcapsules that are monodisperse can refer to such microcapsules that have a narrow distribution of sizes around a mode of the distribution of sizes, such as a mean of the distribution of sizes. In some instances, a set of microcapsules that are monodisperse can have sizes exhibiting a standard deviation of less than 20 percent with respect to a mean of the sizes, such as less than 10 percent or

less than 5 percent. Examples of techniques to form microcapsules can be found in the following references: Tsuei et al., U.S. Pat. No. 5,589,194, entitled "Method of Encapsulation and Microcapsules Produced Thereby;" Tsuei, et al., U.S. Pat. No. 5,433,953, entitled "Microcapsules and Methods for Making Same;" Hatfield, U.S. Pat. No. 4,708,812, entitled "Encapsulation of Phase Change Materials;" and Chen et al., U.S. Pat. No. 4,505,953, entitled "Method for Preparing Encapsulated Phase Change Materials;" the disclosures of which are herein incorporated by reference in their entirities.

Other examples of containment structures include silica particles (e.g., precipitated silica particles, fumed silica particles, and mixtures thereof), zeolite particles, carbon particles (e.g., graphite particles, activated carbon particles, and mixtures thereof), and absorbent materials (e.g., absorbent polymeric materials such as certain cellulosic materials, superabsorbent materials, poly(meth)acrylate materials, metal salts of poly(meth)acrylate materials, and mixtures thereof). For example, a temperature regulating material can include silica particles, zeolite particles, carbon particles, or an absorbent material impregnated with a phase change material.

According to some embodiments of the invention, an elongated member forming a cellulosic fiber can include up to about 100 percent by weight of a temperature regulating material. Typically, an elongated member includes up to about 90 percent by weight of a temperature regulating material. Thus, for example, the elongated member can include up to about 50 percent or up to about 25 percent by weight of the temperature regulating material. For some embodiments of the invention, an elongated member can include from about 1 percent to about 70 percent by weight of a temperature regulating material. Thus, in one embodiment, an elongated member can include from about 1 percent to about 60 percent or from about 5 percent to about 60 percent by weight of a temperature regulating material, and, in other embodiments, an elongated member can include from about 5 percent to about 40 percent, from about 10 percent to about 30 percent, from about 10 percent to about 20 percent, or from about 15 percent to about 25 percent by weight of a temperature regulating material.

A cellulosic fiber in accordance with some embodiments of the invention can have a latent heat that is at least about 1 J/g, such as at least about 2 J/g, at least about 5 J/g, at least about 8 J/g, at least about 11 J/g, or at least about 14 J/g. For example, a cellulosic fiber according to an embodiment of the invention can have a latent heat ranging from about 1 J/g to about 100 J/g, such as from about 5 J/g to about 60 J/g, from about 10 J/g to about 30 J/g, from about 2 J/g to about 20 J/g, from about 5 J/g to about 20 J/g, from about 8 J/g to about 20 J/g, from about 11 J/g to about 20 J/g, or from about 14 J/g to about 20 J/g.

As discussed previously, a cellulosic fiber according to some embodiments of the invention can include a set of elongated members. Various elongated members of the set of elongated members can be formed from the same cellulosic material or different cellulosic materials. In some instances, the set of elongated members can include a first set of elongated members formed from a first cellulosic material that has a temperature regulating material dispersed therein. In addition, the set of elongated members can include a second set of elongated members formed from a second cellulosic material. It is contemplated that the elongated members can be formed from the same cellulosic material, in which case the first and second cellulosic materials will be the same. It is also contemplated that the temperature regulating material can include a polymeric phase change material that provides

adequate mechanical properties. In this case, the polymeric phase change material can be used to form the first set of elongated members without requiring the first cellulosic material.

In general, a cellulosic material can include any cellulose-based polymer (or any mixture of cellulose-based polymers) that has the capability of being formed into an elongated member. A cellulosic material can include a cellulose-based polymer (or a mixture of cellulose-based polymers) having any of various chain structures and including one or more types of monomer units. In particular, a cellulose-based polymer can be a linear polymer or a branched polymer (e.g., star branched polymer, comb branched polymer, or dendritic branched polymer). A cellulose-based polymer can be a homopolymer or a copolymer (e.g., terpolymer, statistical copolymer, random copolymer, alternating copolymer, periodic copolymer, block copolymer, radial copolymer, or graft copolymer). As one of ordinary skill in the art will understand, the reactivity and functionality of a cellulose-based polymer can be altered by addition or replacement of a functional group such as, for example, amine, amide, carboxyl, hydroxyl, ester, ether, epoxide, anhydride, isocyanate, silane, ketone, and aldehyde. Also, a cellulose-based polymer can be capable of crosslinking, entanglement, or hydrogen bonding in order to increase its toughness or its resistance to heat, moisture, or chemicals.

Examples of cellulose-based polymers that can be used to form an elongated member include cellulose and various modified forms of cellulose, such as, for example, cellulose esters (e.g., cellulose acetate, cellulose propionate, cellulose butyrate, cellulose phthalate, and cellulose trimellitate), cellulose nitrate, cellulose phosphate, cellulose ethers (e.g., methyl cellulose, ethyl cellulose, propyl cellulose, and butyl cellulose), other modified forms of cellulose (e.g., carboxy methyl cellulose, hydroxymethyl cellulose, hydroxyethyl cellulose, and cyanoethyl cellulose), and salts or copolymers thereof. Cellulose typically corresponds to a linear homopolymer of D-glucose in which successive monomer units are linked by  $\beta$ -glucoside bonds from an anomeric carbon of one monomer unit to a C-4 hydroxyl group of another monomer unit. Other useful cellulose-based polymers include modified forms of cellulose in which, for example, a certain percentage of hydroxyl groups are replaced by various other types of functional groups. Cellulose acetate typically corresponds to a modified form of cellulose in which a certain percentage of hydroxyl groups are replaced by acetyl groups. The percentage of hydroxyl groups that are replaced can depend upon various processing conditions. In some instances, cellulose acetate can have at least about 92 percent of its hydroxyl groups replaced by acetyl groups, and, in other instances, cellulose acetate can have an average of at least about 2 acetyl groups per monomer unit. For certain applications, a cellulosic material can include cellulose-based polymers having an average molecular chain length in the range of about 300 to about 15,000 monomer units. Thus, in one embodiment, a cellulosic material can include cellulose-based polymers having an average molecular chain length in the range of about 10,000 to about 15,000 monomer units. In other embodiments, a cellulosic material can include cellulose-based polymers having an average molecular chain length in the range of about 300 to about 10,000, such as, for example, from about 300 to about 450 monomer units, from about 450 to about 750 monomer units, or from about 750 to about 10,000 monomer units.

It is contemplated that one or more elongated members can be formed from various other types of polymeric materials.

Thus, in some embodiments of the invention, an elongated member can be formed from any fiber-forming polymer (or any mixture of fiber-forming polymers). Examples polymers that can be used to form an elongated member include polyamides (e.g., Nylon 6, Nylon 6/6, Nylon 12, polyaspartic acid, polyglutamic acid, and so forth), polyamines, polyimides, polyacrylics (e.g., polyacrylamide, polyacrylonitrile, esters of methacrylic acid and acrylic acid, and so forth), polycarbonates (e.g., polybisphenol A carbonate, polypropylene carbonate, and so forth), polydienes (e.g., polybutadiene, polyisoprene, polynorbornene, and so forth), polyepoxides, polyesters (e.g., polyethylene terephthalate, polybutylene terephthalate, polytrimethylene terephthalate, polycaprolactone, polyglycolide, polylactide, polyhydroxybutyrate, polyhydroxyvalerate, polyethylene adipate, polybutylene adipate, polypropylene succinate, and so forth), polyethers (e.g., polyethylene glycol (polyethylene oxide), polybutylene glycol, polypropylene oxide, polyoxymethylene (paraformaldehyde), polytetramethylene ether (polytetrahydrofuran), polyepichlorohydrin, and so forth), polyfluorocarbons, formaldehyde polymers (e.g., urea-formaldehyde, melamine-formaldehyde, phenol formaldehyde, and so forth), natural polymers (e.g., chitosans, lignins, waxes, and so forth), polyolefins (e.g., polyethylene, polypropylene, polybutylene, polybutene, polyoctene, and so forth), polyphenylenes (e.g., polyphenylene oxide, polyphenylene sulfide, polyphenylene ether sulfone, and so forth), silicon containing polymers (e.g., polydimethyl siloxane, polycarbomethyl silane, and so forth), polyurethanes, polyureas, polyvinyls (e.g., polyvinyl butyral, polyvinyl alcohol, esters and ethers of polyvinyl alcohol, polyvinyl acetate, polystyrene, polymethylstyrene, polyvinyl chloride, polyvinyl pyrrolidone, polymethyl vinyl ether, polyethyl vinyl ether, polyvinyl methyl ketone, and so forth), polyacetals, polyarylates, and copolymers (e.g., polyethylene-co-vinyl acetate, polyethylene-co-acrylic acid, polybutylene terephthalate-co-polyethylene terephthalate, polylauryllactam-block-polytetrahydrofuran, and so forth).

According to some embodiments of the invention, one or more elongated members can be formed from a carrier polymeric material. A carrier polymeric material can serve as a carrier for a temperature regulating material as a cellulosic fiber is formed in accordance with some embodiments of the invention. A carrier polymeric material can include a polymer (or a mixture of polymers) that facilitates dispersing or incorporating a temperature regulating material within one or more elongated members. In addition, a carrier polymeric material can facilitate maintaining integrity of one or more elongated members during fiber formation and can provide enhanced mechanical properties to the resulting cellulosic fiber. Desirably, a carrier polymeric material can be selected to be sufficiently non-reactive with a temperature regulating material, such that a desired temperature stabilizing range is maintained when the temperature regulating material is dispersed within the carrier polymeric material.

A carrier polymeric material can be used in conjunction with, or as an alternative to, a cellulosic material when forming one or more elongated members. In some instances, a carrier polymeric material can serve as a containment structure to facilitate handling of a phase change material while also offering a degree of protection to the phase change material during formation of a cellulosic fiber or a product made therefrom. During formation of a cellulosic fiber, a carrier polymeric material can be provided as a solid in any of various forms (e.g., bulk form, powders, pellets, granules, flakes, and so forth) and can have a temperature regulating material dispersed therein. Thus, for example, powders or pellets formed from the carrier polymeric material having the tem-

perature regulating material dispersed therein can be mixed with a cellulosic material to form a blend, which is used to form one or more elongated members. It is contemplated that a carrier polymeric material can be provided as a liquid in any of various forms (e.g., molten form, dissolved in a solvent, and so forth) and can have a temperature regulating material dispersed therein. It is also contemplated that a cellulosic material can serve as a carrier polymeric material. For example, a cellulosic material having a temperature regulating material dispersed therein can be mixed with the same or a different cellulosic material to form a blend, which is used to form one or more elongated members.

For certain applications, a carrier polymeric material can include a polymer (or a mixture of polymers) that is compatible or miscible with or has an affinity for a temperature regulating material. Such affinity can depend on a number of factors, such as, for example, similarity of solubility parameters, polarities, hydrophobic characteristics, or hydrophilic characteristics of the carrier polymeric material and the temperature regulating material. An affinity for a temperature regulating material can facilitate dispersion of the temperature regulating material in an intermediate molten, liquid, or dissolved form of a carrier polymeric material during formation of a cellulosic fiber. Ultimately, such affinity can facilitate incorporation of more uniform or greater amounts (e.g., higher loading levels) of a phase change material in the cellulosic fiber.

For embodiments of the invention where a temperature regulating material includes a containment structure such as microcapsules, a carrier polymeric material can include a polymer (or a mixture of polymers) having an affinity for the containment structure in conjunction with, or as an alternative to, its affinity for a phase change material. For example, if the temperature regulating material includes various microcapsules containing the phase change material, a polymer (or a mixture of polymers) can be selected based on its affinity for the microcapsules (e.g., for a material of which the microcapsules are formed). In some instances, the carrier polymeric material can include the same or a similar polymer as one forming the microcapsules. Thus, for example, if the microcapsules include nylon shells, the carrier polymeric material can be selected to include nylon. Such affinity for the microcapsules can facilitate dispersion of the microcapsules containing the phase change material in an intermediate molten, liquid, or dissolved form of the carrier polymeric material and, thus, facilitates incorporation of more uniform or greater amounts of the phase change material in a cellulosic fiber.

In some instances, a carrier polymeric material can include a polymer (or a mixture of polymers) that has a partial affinity for a temperature regulating material. For example, the carrier polymeric material can include a polymer (or a mixture of polymers) that is semi-miscible with the temperature regulating material. Such partial affinity can be adequate to facilitate dispersion of the temperature regulating material within the carrier polymeric material at higher temperatures and shear conditions. At lower temperatures and shear conditions, such partial affinity can allow the temperature regulating material to separate out. If a phase change material in a raw form is used, such partial affinity can lead to insolubilization of the phase change material and increased phase change material domain formation within the carrier polymeric material and within the resulting cellulosic fiber. Domain formation can lead to improved thermal regulating properties by facilitating transition of the phase change material between two states. In addition, domain formation can serve to reduce or prevent loss or leakage of the phase change material from the cellulosic fiber during fiber formation or during end use.

For example, certain phase change materials such as paraffinic hydrocarbons can be compatible with polyolefins or copolymers of polyolefins at lower concentrations of the phase change materials or when the temperature is above a critical solution temperature. Thus, for example, mixing of a paraffinic hydrocarbon (or a mixture of paraffinic hydrocarbons) and polyethylene or polyethylene-co-vinyl acetate can be achieved at higher temperatures to produce a substantially homogenous blend that can be easily controlled, pumped, and processed in connection with fiber formation. Once the blend has cooled, the paraffinic hydrocarbon can become insoluble and can separate out into distinct domains within a solid material. These domains can allow for pure melting or crystallization of the paraffinic hydrocarbon for an improved thermal regulating property. In addition, these domains can serve to reduce or prevent loss or leakage of the paraffinic hydrocarbon. The solid material having the domains dispersed therein can be processed to form powders or pellets, which can be mixed with a cellulosic material to form a cellulosic fiber.

According to some embodiments of the invention, a carrier polymeric material can include polyethylene-co-vinyl acetate having from about 5 percent to about 90 percent by weight of vinyl acetate, such as, for example, from about 5 percent to about 50 percent by weight of vinyl acetate or from about 18 percent to about 25 percent by weight of vinyl acetate. This content of vinyl acetate can allow for improved temperature miscibility control when mixing a paraffinic hydrocarbon and the polyethylene-co-vinyl acetate to form a blend. In particular, this vinyl acetate content can allow for excellent miscibility at higher temperatures, thus facilitating processing stability and control due to homogeneity of the blend. At lower temperatures (e.g., room temperature or normal commercial fabric use temperatures), the polyethylene-co-vinyl acetate is semi-miscible with the paraffinic hydrocarbon, thus allowing for separation and micro-domain formation of the paraffinic hydrocarbon.

Other polymers that can be included in a carrier polymeric material include high-density polyethylenes having a melt index in the range of about 4 to about 36 g/10 min (e.g., high-density polyethylenes having melt indices of 4, 12, and 36 g/10 min, available from Sigma-Aldrich Corp., St. Louis, Mo.), modified forms of high-density polyethylenes (e.g., Fusabond® E MB100D, available from DuPont Inc., Wilmington, Del.), and modified forms of ethylene propylene rubber (e.g., Fusabond® N MF416D, available from DuPont Inc., Wilmington, Del.). As one of ordinary skill in the art will understand, a melt index typically refers to a measure of the flow characteristics of a polymer (or a mixture of polymers) and inversely correlates with a molecular weight of the polymer (or the mixture of polymers). For polar phase change materials (e.g., polyethylene glycols, polytetramethylene glycols, and their homologues), a carrier polymeric material can include a polar polymer (or a mixture of polar polymers) to facilitate dispersion of the phase change materials. Thus, for example, the carrier polymeric material can include copolymers of polyesters, such as, for example, polybutylene terephthalate-block-polytetramethylene glycols (e.g., Hytrel® 3078, 5544, and 8238, available from DuPont Inc., Wilmington, Del.), and copolymers of polyamides, such as, for example, polyamide-block-polyethers (e.g., Pebax® 2533, 4033, 5533, 7033, MX 1205, and MH 1657, available from ATOFINA Chemicals, Inc., Philadelphia, Pa.).

As discussed previously, a cellulosic material can serve as a carrier polymeric material in some embodiments of the invention. For example, certain phase change materials such as polyethylene glycols can be compatible with cellulose-

based polymers in a solution. In particular, mixing of a polyethylene glycol (or a mixture of polyethylene glycols) and cellulose or cellulose acetate can be achieved to produce a substantially homogenous blend as described in the article of Guo et al., "Solution Miscibility and Phase-Change Behavior of a Polyethylene Glycol-Diacetate Cellulose Composite," *Journal of Applied Polymer Science*, Vol. 88, 652-658 (2003), the disclosure of which is incorporated herein by reference in its entirety. The polyethylene glycol can form distinct domains within a resulting solid material and can undergo a transition between two solid states within these domains. The solid material having the domains dispersed therein can be processed to form powders or pellets, which can be mixed with a cellulosic material to form a cellulosic fiber.

According to some embodiments of the invention, a carrier polymeric material can include a low molecular weight polymer (or a mixture of low molecular weight polymers). As discussed previously, some polymers can be provided in various forms having different molecular weights. Accordingly, a low molecular weight polymer can refer to a low molecular weight form of the polymer. For example, a polyethylene having a number average molecular weight of about 20,000 (or less) can be used as a low molecular weight polymer in an embodiment of the invention. A low molecular weight polymer typically has a low viscosity when heated to form a melt, which low viscosity can facilitate dispersion of a temperature regulating material in the melt. It is contemplated that a desired molecular weight or range of molecular weights of a low molecular weight polymer can depend upon the particular polymer selected (e.g., polyethylene) or upon the method or equipment used to disperse a temperature regulating material in a melt of the low molecular weight polymer.

According to another embodiment of the invention, a carrier polymeric material can include a mixture of a low molecular weight polymer and a high molecular weight polymer. A high molecular weight polymer can refer to a high molecular weight form of the polymer. A high molecular weight polymer typically has enhanced mechanical properties but can have a high viscosity when heated to form a melt. In some instances, a low molecular weight polymer and a high molecular weight polymer can be selected to have an affinity for one another. Such affinity can facilitate forming a blend of the low molecular weight polymer, the high molecular weight polymer, and a temperature regulating material during fiber formation and can facilitate incorporation of more uniform or greater amounts of a phase change material in a cellulosic fiber. According to some embodiments of the invention, a low molecular weight polymer can serve as a compatibilizing link between a high molecular weight polymer and a temperature regulating material to facilitate incorporating the temperature regulating material in a cellulosic fiber.

Cellulosic fibers in accordance with various embodiments of the invention can be formed using various methods, including, for example, a solution spinning process (wet or dry). In a solution spinning process, one or more cellulosic materials and one or more temperature regulating materials can be delivered to orifices of a spinneret. As one of ordinary skill in the art will understand, a spinneret typically refers to a portion of a fiber forming apparatus that delivers molten, liquid, or dissolved materials through orifices for extrusion into an outside environment. A spinneret typically includes from about 1 to about 500,000 orifices per meter of length of the spinneret. A spinneret can be implemented with holes drilled or etched through a plate or with any other structure capable of issuing desired fibers.

A cellulosic material can be initially provided in any of various forms, such as, for example, sheets of cellulose, wood

pulp, cotton linters, and other sources of substantially purified cellulose. Typically, a cellulosic material is dissolved in a solvent prior to passing through the orifices of the spinneret. In some instances, the cellulosic material can be processed (e.g., chemically treated) prior to dissolving the cellulosic material in the solvent. For example, the cellulosic material can be immersed in a basic solution (e.g., caustic soda), squeezed through rollers, and then shredded to form crumbs. The crumbs can then be treated with carbon disulfide to form cellulose xanthate. As another example, the cellulosic material can be mixed with a solution of glacial acetic acid, acetic anhydride, and a catalyst and then aged to form cellulose acetate, which can precipitate from the solution in the form of flakes.

The composition of a solvent used to dissolve a cellulosic material can vary depending upon a desired application of the resulting cellulosic fibers. For example, crumbs of cellulose xanthate as discussed above can be dissolved in a basic solvent (e.g., caustic soda or 2.8 percent sodium hydroxide solution) to form a viscous solution. As another example, precipitated flakes of cellulose acetate as discussed above can be dissolved in acetone to form a viscous solution. Various other types of solvents can be used, such as, for example, a solution of amine oxide or a cuprammonium solution. In some instances, the resulting viscous solution can be filtered to remove any undissolved cellulosic material.

During formation of cellulosic fibers, a temperature regulating material can be mixed with a cellulosic material to form a blend. As a result of mixing, the temperature regulating material can be dispersed within and at least partially enclosed by the cellulosic material. The temperature regulating material can be mixed with the cellulosic material at various stages of fiber formation. Typically, the temperature regulating material is mixed with the cellulosic material prior to passing through the orifices of the spinneret. In particular, the temperature regulating material can be mixed with the cellulosic material prior to or after dissolving the cellulosic material in a solvent. For example, the temperature regulating material can include microcapsules containing a phase change material, and the microcapsules can be dispersed in a viscous solution of the dissolved cellulosic material. In some instances, the temperature regulating material can be mixed with the viscous solution just prior to passing through the orifices of the spinneret.

According to some embodiments of the invention, cellulosic fibers can be formed using a carrier polymeric material. For example, the cellulosic fibers can be formed using powders or pellets formed from the carrier polymeric material having a temperature regulating material dispersed therein. In some instances, the powders or pellets can be formed from a solidified melt mixture of the carrier polymeric material and the temperature regulating material. It is contemplated that the powders or pellets can be initially formed from the carrier polymeric material and can be impregnated or imbibed with the temperature regulating material. It is also contemplated that the powders or pellets can be formed from a dried solution of the carrier polymeric material and the temperature regulating material. During formation of the cellulosic fibers, the powders or pellets can be mixed with a cellulosic material to form a blend at various stages of fiber formation. Typically, the powders or pellets are mixed with the cellulosic material prior to passing through the orifices of the spinneret.

For certain applications, cellulosic fibers can be formed as multi-component fibers. In particular, a first cellulosic material can be mixed with a temperature regulating material to form a blend. The blend and a second cellulosic material can be combined and directed through the orifices of the spinneret

31

in a particular configuration to form respective elongated members of the cellulosic fibers. For example, the blend can be directed through the orifices to form core members or island members, while the second cellulosic material can be directed through the orifices to form sheath members or sea members. Prior to passing through the orifices, the first cellulosic material and the second cellulosic material can be dissolved in the same solvent or different solvents. Portions of the temperature regulating material that are not enclosed by the first cellulosic material can be enclosed by the second cellulosic material upon emerging from the spinneret to reduce or prevent loss or leakage of the temperature regulating material from the resulting cellulosic fibers. It is contemplated that the first cellulosic material need not be used for certain applications. For example, the temperature regulating material can include a polymeric phase change material having a desired transition temperature and providing adequate mechanical properties when incorporated in the cellulosic fibers. The polymeric phase change material and the second cellulosic material can be combined and directed through the orifices of the spinneret in a particular configuration to form respective elongated members of the cellulosic fibers. For example, the polymeric phase change material can be directed through the orifices to form core members or island members, while the second cellulosic material can be directed through the orifices to form sheath members or sea members.

Upon emerging from the spinneret, one or more cellulosic materials typically solidify to form cellulosic fibers. In a wet solution spinning process, the spinneret can be submerged in a coagulation or spinning bath (e.g., a chemical bath), such that, upon exiting the spinneret, one or more cellulosic materials can precipitate and form solid cellulosic fibers. The composition of a spinning bath can vary depending upon a desired application of the resulting cellulosic fibers. For example, the spinning bath can be water, an acidic solution (e.g., a weak acid solution including sulfuric acid), or a solution of amine oxide. In a dry solution spinning process, one or more cellulosic materials can emerge from the spinneret in warm air and solidify due to a solvent (e.g., acetone) evaporating in the warm air.

After emerging from the spinneret, cellulosic fibers can be drawn or stretched utilizing a godet or an aspirator. For example, cellulosic fibers emerging from the spinneret can form a vertically oriented curtain of downwardly moving cellulosic fibers that are drawn between variable speed godet rolls before being wound on a bobbin or cut into staple fiber. Cellulosic fibers emerging from the spinneret can also form a horizontally oriented curtain within a spinning bath and can be drawn between variable speed godet rolls. As another example, cellulosic fibers emerging from the spinneret can be at least partially quenched before entering a long, slot-shaped air aspirator positioned below the spinneret. The aspirator can introduce a rapid, downwardly moving air stream produced by compressed air from one or more air aspirating jets. The air stream can create a drawing force on the cellulosic fibers, causing them to be drawn between the spinneret and the air jet and attenuating the cellulosic fibers. During this portion of fiber formation, one or more cellulosic materials forming the cellulosic fibers can be solidifying. It is contemplated that drawing or stretching of cellulosic fibers can occur before or after drying the cellulosic fibers.

Once formed, cellulosic fibers can be further processed for various fiber applications. In particular, cellulosic fibers in accordance with various embodiments of the invention can be used or incorporated in various products to provide thermal regulating properties to those products. For example, cellulosic fibers can be used in textiles (e.g., fabrics), apparel (e.g.,

32

outdoor clothing, drysuits, and protective suits), footwear (e.g., socks, boots, and insoles), medical products (e.g., thermal blankets, therapeutic pads, incontinent pads, and hot/cold packs), personal hygiene products (e.g., diapers, tampons, and absorbent wipes or pads for body care and for baby care), cleaning products (e.g., absorbent wipes or pads for household cleaning, for commercial cleaning, and for industrial cleaning), containers and packagings (e.g., beverage/food containers, food warmers, seat cushions, and circuit board laminates), buildings (e.g., insulation in walls or ceilings, wallpaper, curtain linings, pipe wraps, carpets, and tiles), appliances (e.g., insulation in house appliances), technical products (e.g., filter materials), and other products (e.g., automotive lining material, furnishings, sleeping bags, and bedding).

In some instances, cellulosic fibers can be subjected to, for example, woven, non-woven, knitting, or weaving processes to form various types of plaited, braided, twisted, felted, knitted, woven, or non-woven fabrics. The resulting fabrics can include a single layer formed from the cellulosic fibers, or can include multiple layers such that at least one of those layers is formed from the cellulosic fibers. For example, cellulosic fibers can be wound on a bobbin or spun into a yarn and then utilized in various conventional knitting or weaving processes. As another example, cellulosic fibers can be randomly laid on a forming surface (e.g., a moving conveyor screen belt such as a Fourdrinier wire) to form a continuous, non-woven web of cellulosic fibers. In some instances, cellulosic fibers can be cut into short staple fibers prior to forming the web. One potential advantage of employing staple fibers is that a more isotropic non-woven web can be formed, since the staple fibers can be oriented in the web more randomly than longer or uncut fibers (e.g., continuous fibers in the form of a tow). The web can then be bonded using any conventional bonding process (e.g., a spunbond process) to form a stable, non-woven fabric for use in manufacturing various textiles. An example of a bonding process involves lifting the web from a moving conveyor screen belt and passing the web through two heated calender rolls. One, or both, of the rolls can be embossed to cause the web to be bonded in numerous spots. Carded (e.g., air carded) webs, needle-punched webs, spun-laced webs, air-laid webs, wet-laid webs, as well as spun-laid webs can be formed from cellulosic fibers in accordance with some embodiments of the invention.

It is contemplated that fabrics can be formed from cellulosic fibers including two or more different temperature regulating materials. According to some embodiments of the invention, such combination of temperature regulating materials can exhibit two or more distinct transition temperatures. For example, a fabric for use in a glove can be formed from cellulosic fibers that each includes phase change materials A and B. Phase change material A can have a melting point of about 5° C., and phase change material B can have a melting point of about 75° C. This combination of phase change materials in the cellulosic fibers can provide the glove with improved thermal regulating properties in cold environments (e.g., outdoor use during winter conditions) as well as warm environments (e.g., when handling heated objects such as oven trays). In addition, fabrics can be formed from two or more types of fibers that differ in some fashion (e.g., two or more types of cellulosic fibers with different configurations or cross-sectional shapes or formed so as to include different temperature regulating materials). For example, a fabric can be formed with a certain percentage of cellulosic fibers including phase change material A and a remaining percentage of cellulosic fibers including phase change material B.

This combination of cellulosic fibers can provide the fabric with improved thermal regulating properties in different environments (e.g., cold and warm environments). As another example, a fabric can be formed with a certain percentage of cellulosic fibers including a phase change material and a remaining percentage of cellulosic fibers lacking a phase change material. In this example, the percentage of the cellulosic fibers including the phase change material can range from about 10 percent to about 99 percent by weight, such as from about 30 percent to about 80 percent or from about 40 percent to about 70 percent. As a further example, a fabric can be formed with a certain percentage of cellulosic fibers including a phase change material and a remaining percentage of other fibers (e.g., synthetic fibers formed from other polymers) that either include or lack a phase change material. In this example, the percentage of the cellulosic fibers can also range from about 10 percent to about 99 percent by weight, such as from about 30 percent to about 80 percent or from about 40 percent to about 70 percent.

A resulting fabric in accordance with some embodiments of the invention can have a latent heat that is at least about 1 J/g, such as at least about 2 J/g, at least about 5 J/g, at least about 8 J/g, at least about 11 J/g, or at least about 14 J/g. For example, a fabric according to an embodiment of the invention can have a latent heat ranging from about 1 J/g to about 100 J/g, such as from about 5 J/g to about 60 J/g, from about 10 J/g to about 30 J/g, from about 2 J/g to about 20 J/g, from about 5 J/g to about 20 J/g, from about 8 J/g to about 20 J/g, from about 11 J/g to about 20 J/g, or from about 14 J/g to about 20 J/g.

In addition, a resulting fabric in accordance with some embodiments of the invention can exhibit other desirable properties. For example, a fabric (e.g., a non-woven fabric) according to an embodiment of the invention can have one or more of the following properties: (1) a moisture absorbency that is at least 10 gram/gram, such as from about 12 gram/gram to about 35 gram/gram, from about 15 gram/gram to about 30 gram/gram, or from about 18 gram/gram to about 25 gram/gram (expressed as a ratio of a weight of absorbed moisture relative to a moisture-free weight of the fabric under a particular environmental condition); (2) a sink time that is from about 2 seconds to about 60 seconds, such as from about 3 seconds to about 20 seconds or from about 4 seconds to about 10 seconds; (3) a tensile strength that is from about 13 cN/tex to about 40 cN/tex, such as from about 16 cN/tex to about 30 cN/tex or from about 18 cN/tex to about 25 cN/tex; (4) an elongation at break that is from about 10 percent to about 40 percent, such as from about 14 percent to about 30 percent or from about 17 percent to about 22 percent; (5) a shrinkage in boiling water that is from about 0 percent to about 6 percent, such as from about 0 percent to about 4 percent or from about 0 percent to about 3 percent; and (6) a specific weight that is from about 10 g/m<sup>2</sup> to about 500 g/m<sup>2</sup>, such as about 15 g/m<sup>2</sup> to about 400 g/m<sup>2</sup> or from about 40 g/m<sup>2</sup> to about 150 g/m<sup>2</sup>.

At this point, one of ordinary skill in the art can appreciate a number of advantages associated with various embodiments of the invention. For example, cellulosic fibers in accordance with various embodiments of the invention can provide improved thermal regulating properties along with high moisture absorbency. Such combination of properties allows for an improved level of comfort when the cellulosic fibers are incorporated in products such as apparel, footwear, personal hygiene products, and medical products. A cellulosic fiber in accordance with some embodiments of the invention can include a high loading level of a phase change material within a first set of elongated members. In some instances, such high

loading level can be provided because a second set of elongated members can surround the first set of elongated members. The second set of elongated members can compensate for any deficiencies (e.g., mechanical or moisture absorbency deficiencies) of the first set of elongated members. Moreover, the second set of elongated members can include a cellulosic material selected to improve the cellulosic fiber's overall mechanical properties, moisture absorbency, and processability (e.g., by facilitating its formation via a solution spinning process). By surrounding the first set of elongated members, the second set of elongated members can serve to enclose the phase change material within the cellulosic fiber to reduce or prevent loss or leakage of the phase change material.

15

## EXAMPLES

The following examples are provided as a guide for a practitioner of ordinary skill in the art. These examples should not be construed as limiting the invention, as the examples merely provide specific methodology useful in understanding and practicing some embodiments of the invention.

### Example 1

Three sets of cellulosic fibers were formed. A first set of cellulosic fibers was used as a control set. For the first set of cellulosic fibers, 8.00 g of N-methyl morpholine oxide solvent (97 percent NMMO, available from Aldrich Chemical Co., Milwaukee, Wis.), 1.00 g of microcrystalline cellulose (available from Aldrich Chemical Co., Milwaukee, Wis.), and 1.00 g of deionized water were combined in a 20 ml glass vial to yield a solution with 10 percent by weight of cellulose. The vial was placed in a 125° C. oven and periodically mixed until its contents were homogenously mixed. The contents were then poured into a preheated 10 ml syringe and slowly squeezed into a coagulation bath of warm, stirred water to form the first set of cellulosic fibers.

For a second set of cellulosic fibers, 0.90 g of deionized water and 0.20 g of water-wetted microcapsules containing a phase change material (microencapsulated paraffin PCM, 120 J/g latent heat, 33° C. melting point, 50 percent microcapsules, available from Ciba Specialty Chemical Co., Bradford, United Kingdom) were combined in a 20 ml glass vial. Next, 8.00 g of N-methyl morpholine oxide solvent (97 percent NMMO, available from Aldrich Chemical Co., Milwaukee, Wis.) and 0.90 g of microcrystalline cellulose (available from Aldrich Chemical Co., Milwaukee, Wis.) were added to yield a solution with 10 percent by weight of solids. The solids included a 90/10 weight ratio of cellulose/microcapsules containing the phase change material. The vial was placed in a 125° C. oven and periodically mixed until its contents were homogenously mixed. The contents were then poured into a preheated 10 ml syringe and slowly squeezed into a coagulation bath of warm, stirred water to form lyocell-type cellulosic fibers with enhanced reversible thermal properties.

For a third set of cellulosic fibers, 0.80 g of deionized water and 0.31 g of water-wetted microcapsules containing a phase change material (microencapsulated paraffin PCM, 154 J/g latent heat, 31° C. melting point, 32 percent microcapsules, available from J&C Microchem Inc., Korea) were combined in a 20 ml glass vial. Next, 8.00 g of N-methyl morpholine oxide solvent (97 percent NMMO, available from Aldrich Chemical Co., Milwaukee, Wis.) and 0.90 g of microcrystalline cellulose (available from Aldrich Chemical Co., Milwaukee, Wis.) were added to yield a solution with 10 percent by

weight of solids. The solids included a 90/10 weight ratio of cellulose/microcapsules containing the phase change material. The vial was placed in a 125° C. oven and periodically mixed until its contents were homogenously mixed. The contents were then poured into a preheated 10 ml syringe and slowly squeezed into a coagulation bath of warm, stirred water to form lyocell-type cellulosic fibers with enhanced reversible thermal properties.

The three sets of cellulosic fibers were filtered and dried, and thermal measurements were made using Differential Scanning Calorimetry (DSC). Table 4 sets forth results of these thermal measurements for the three sets of cellulosic fibers.

TABLE 4

| Cellulosic Fibers       | Melting Point (° C.) | Latent Heat (J/g) |
|-------------------------|----------------------|-------------------|
| First Set (Control Set) | None                 | None              |
| Second Set              | 31.3                 | 9.8               |
| Third Set               | 32.4                 | 13.5              |

## Example 2

A suspension was formed by adding in (with stirring) 100.0 kilograms of water and then 5.2 kilograms of a 50 percent

TABLE 5-continued

| 5            | Concentration of mPCM (%) | Latent Heat (J/g) | Linear Density (decitex) | Tenacity (cN/tex) | Elongation (%) |
|--------------|---------------------------|-------------------|--------------------------|-------------------|----------------|
| Sample set B |                           |                   |                          |                   |                |
|              |                           |                   |                          |                   |                |
| 10           | 1                         | 0                 | 0                        | 1.7               | 21.7           |
|              | 2                         | 10                | 11.4                     | 1.6               | 16.0           |
|              | 3                         | 20                | 19.4                     | 1.5               | 15.1           |
|              | 4                         | 0                 | 0                        | 1.2               | 22.3           |
|              | 5                         | 10                | 11.9                     | 1.2               | 16.8           |
|              | 6                         | 20                | 21.6                     | 1.2               | 13.4           |
|              | 7                         | 30                | 27.7                     | 1.6               | 13.9           |
| 15           |                           |                   |                          |                   | 12             |

## Example 3

Two sets of viscose-type cellulosic fibers were formed. A first set of cellulosic fibers was used as a control set, and included TiO<sub>2</sub> as a dulling agent. A second set of cellulosic fibers included microcapsules containing a phase change material (mPCM), but lacked TiO<sub>2</sub>. Table 6 sets forth properties of the two sets of cellulosic fibers. As can be appreciated with reference to Table 6, the second set of cellulosic fibers exhibited enhanced reversible thermal properties along with a dull appearance (without requiring the use of TiO<sub>2</sub>).

TABLE 6

| Cellulosic Fibers       | Amount of mPCM (%) | Amount of TiO <sub>2</sub> (%) | Linear Density (decitex) | Staple Cut Length (mm) | Latent Heat (J/g) |
|-------------------------|--------------------|--------------------------------|--------------------------|------------------------|-------------------|
| First Set (Control Set) | 0.0                | Dull                           | 0.6-1.0                  | 1.7                    | 40                |
| Second Set              | 15.0               | Dull                           | 0.0                      | 1.7                    | 40                |

NaOH/water solution to 100.0 kilograms of microcapsules containing a phase change material (mPCM, polyacrylic shell microcapsules containing octadecane, 175 J/g latent heat, 45 percent microcapsules, available from Ciba Specialty Chemical Co., Bradford, United Kingdom). The suspension contained 21.95 percent by weight of the microcapsules at a pH of about 12.8. The suspension was metered into a 9.1 percent cellulose solution to yield various sample sets with different mPCM concentrations, and then spun into cellulosic fibers as set forth in Table 5 below.

TABLE 5

| Concentration of mPCM (%) | Latent Heat (J/g) | Linear Density (decitex) | Tenacity (cN/tex) | Elongation (%) |
|---------------------------|-------------------|--------------------------|-------------------|----------------|
| Sample set A              |                   |                          |                   |                |
| 1                         | 5                 | 6.9                      | 17.9              | 13.6           |
| 2                         | 10                | 14                       | 17.0              | 14.3           |
| 3                         | 5                 | 7.7                      | 4.3               | 15.2           |
| 4                         | 10                | 14.5                     | 4.5               | 13.8           |
| 5                         | 5                 | 7.2                      | 1.8               | 17.9           |
| 6                         | 10                | 14                       | 1.5               | 17.4           |
| 7                         | 5                 | 6.8                      | 0.9               | 18.6           |
| 8                         | 8                 | 10.7                     | 0.9               | 12.5           |
|                           |                   |                          | 17.0              | 11.6           |

Various non-woven fabrics were formed using either the second set of cellulosic fibers alone or as a blend along with standard viscose-type cellulosic fibers. The non-woven fabrics were formed using a standard viscose needlepunch non-woven line. The line was operated at speeds of about 1.5 to 2.5 meters/minute. Table 7 sets forth properties of the non-woven fabrics.

TABLE 7

| 50 | Non-woven Fabrics                               | Fabric Weight (g/m <sup>2</sup> ) | Latent Heat (J/g) |
|----|-------------------------------------------------|-----------------------------------|-------------------|
| 55 | 100% of Second Set                              |                                   | 13.0-13.2         |
|    | 100% of Second Set (needled non-woven)          | 180 g/m <sup>2</sup>              | 12.8-13.2         |
|    | 50% of Second Set (blend with standard viscose) |                                   | 6.8-7.7           |
|    | 50% of Second Set (needled non-woven)           | 70 g/m <sup>2</sup>               | 6.6-7.7           |
|    | 50% of Second Set (needled non-woven)           | 175 g/m <sup>2</sup>              | 6.6-7.7           |
| 60 | 30% of Second Set (blend with standard viscose) |                                   | 4.3-4.8           |
|    | 30% of Second Set (needled non-woven)           | 80 g/m <sup>2</sup>               | 4.0-4.8           |
| 65 | 30% of Second Set (needled non-woven)           | 160 g/m <sup>2</sup>              | 4.0-4.8           |

Two spunlace, non-woven fabric samples were formed. A first fabric sample was formed from 100 percent viscose-type cellulosic fibers that included microcapsules containing a phase change material (mPCM). A second fabric sample was formed from 100 percent standard viscose-type cellulosic fibers, and was used as a control. The two fabric samples were formed using a standard pilot line, which was operated at a speed of about 10 meters/minute and at pressures of 14, 50, 60, 70/60, and 70 bar on the line. There was no observable difference in the manufacturability of the two fabric samples.

The two fabric samples were then subjected to various measurements in accordance with standard test methods. Measurements for weight were performed in accordance the European Disposables and Nonwoven Association ("EDANA") Test Method ERT40.3-90. Measurements for thickness were performed with a gauge pressure of 0.8 kPa (or 0.8 g/cm<sup>2</sup>) and a foot area of 6.12 cm<sup>2</sup>. Measurements for tensile strength and elongation were performed in accordance with EDANA Test Method ERT20.2-89, and measurements for absorption and sink times were performed in accordance with STL Test Method and European Pharmacopeia Test Methods. Table 8 sets forth results of these measurements. In Table 8, MD refers to a longitudinal or machine direction, while TD refers to a transverse direction. As can be appreciated with reference to Table 8, the first fabric sample generally exhibited properties that were comparable to, or superior to, those of the second fabric sample.

TABLE 8

| Measurement                                          | Sample 1<br>(with mPCM) | Sample 2<br>(Control) |
|------------------------------------------------------|-------------------------|-----------------------|
| Fabric Weight (grams)                                | 50.4                    | 53.0                  |
| Fabric Thickness (mm)                                | 0.4                     | 0.4                   |
| Fabric Density (g/cm <sup>3</sup> )                  | 0.126                   | 0.133                 |
| Fabric Absorbency, water pickup gram/gram, MD        | 11.8                    | 9.4                   |
| Fabric Absorbency, water pickup gram/gram, TD        | 13.2                    | 10.2                  |
| Fabric Absorbency, water pickup gram/gram, MD + TD   | 12.5                    | 9.8                   |
| Fabric Absorbency, water retained gram/gram, MD      | 10.7                    | 9.2                   |
| Fabric Absorbency, water retained gram/gram, TD      | 11.0                    | 8.7                   |
| Fabric Absorbency, water retained gram/gram, MD + TD | 10.9                    | 8.9                   |
| Fabric Absorbency, sink time (sec)                   | 10.5-7.0                | 5.0-1.5               |
| Fabric Tensile Strength, MD dry, N/5 cm              | 63.8                    | 102.8                 |
| Fabric Elongation at Break, MD dry %                 | 38                      | 24                    |
| Fabric Tensile Strength, TD dry, N/5 cm              | 9.2                     | 18.9                  |
| Fabric Elongation at Break, TD dry %                 | 135                     | 100                   |
| Fabric Tenacity, MD + TD, dry CN/tex                 | 2.9                     | 4.6                   |
| Fabric Tensile Strength, MD wet, N/5 cm              | 25.7                    | 45.5                  |
| Fabric Elongation at break, MD wet %                 | 32                      | 29                    |
| Fabric Tensile Strength, TD wet, N/5 cm              | 7.8                     | 12.2                  |
| Fabric Elongation at Break, TD wet %                 | 80                      | 82                    |
| Fabric Tenacity, MD + TD, wet CN/tex                 | 1.33                    | 2.2                   |

| Measurement                     | Sample 1<br>(with mPCM) | Sample 2<br>(Control) |
|---------------------------------|-------------------------|-----------------------|
| Fabric % Tenacity loss in water | 54                      | 53                    |

A practitioner of ordinary skill in the art should require no additional explanation in developing the cellulosic fibers described herein but may nevertheless find some helpful guidance by examining the book of Kadolph et al., "Textiles," Chapter 7—Manufactured Regenerated Fibers (8th ed., Prentice-Hall, Inc. 1998) and the patents of Frankham et al., entitled "Tampon Production," U.S. Pat. No. 5,686,034; Wilkes et al., entitled "Cellulose Fibre Compositions," U.S. Pat. No. 6,333,108; Fischer et al., entitled "Manufacture of Viscose and of Articles Therefrom," U.S. Pat. No. 6,538,130; Poggi et al., entitled "Method for Viscose Production," U.S. Pat. No. 6,392,033; and Hills, entitled "Method of Making Plural Component Fibers," U.S. Pat. No. 5,162,074, the disclosures of which are incorporated herein by reference in their entireties. A practitioner of ordinary skill in the art may also find some helpful guidance by examining the patents of Hartmann, entitled "Stable Phase Change Materials For Use In Temperature Regulating Synthetic Fibers, Fabrics And Textiles," U.S. Pat. No. 6,689,466; and Hartmann et al., entitled "Melt Spinnable Concentrate Pellets Having Enhanced Reversible Thermal Properties," U.S. Pat. No. 6,793,856, the disclosures of which are incorporated in by reference in their entireties.

Each of the patent applications, patents, publications, and other published documents mentioned or referred to in this specification is herein incorporated by reference in its entirety, to the same extent as if each individual patent application, patent, publication, and other published document was specifically and individually indicated to be incorporated by reference.

While the invention has been described with reference to the specific embodiments thereof, it should be understood by those skilled in the art that various changes may be made and equivalents may be substituted without departing from the true spirit and scope of the invention as defined by the appended claims. In addition, many modifications may be made to adapt a particular situation, material, composition of matter, method, process step or steps, to the objective, spirit and scope of the invention. All such modifications are intended to be within the scope of the claims appended hereto. In particular, while the methods disclosed herein have been described with reference to particular operations performed in a particular order, it will be understood that these operations may be combined, sub-divided, or re-ordered to form an equivalent method without departing from the teachings of the invention. Accordingly, unless specifically indicated herein, the order and grouping of the operations are not limitations of the invention.

What is claimed is:

1. A cellulosic fiber comprising:  
a fiber body including a cellulosic material and a plurality of microcapsules dispersed in the cellulosic material, the plurality of microcapsules containing a phase change material having a latent heat of at least 40 J/g and a transition temperature in the range of 0° C. to 100° C., the phase change material providing thermal regulation based on at least one of absorption and release of the latent heat at the transition temperature, wherein the

**39**

- cellulosic fiber includes from 5 percent to 40 percent by weight of the plurality of microcapsules containing the phase change material.
2. The cellulosic fiber of claim 1, wherein the cellulosic material includes one of cellulose and cellulose acetate.
  3. The cellulosic fiber of claim 1, wherein the plurality of microcapsules have sizes in the range 0.1 to 20 microns.
  4. The cellulosic fiber of claim 1, wherein the plurality of microcapsules are monodisperse with respect to sizes of the plurality of microcapsules.
  5. The cellulosic fiber of claim 1, wherein the latent heat of the phase change material is in the range of 60 J/g to 400 J/g.
  6. The cellulosic fiber of claim 1, wherein the transition temperature of the phase change material is in the range of 0° C. to 50° C.
  7. The cellulosic fiber of claim 1, wherein the phase change material includes a paraffinic hydrocarbon.
  8. The cellulosic fiber of claim 1, wherein the phase change material includes a polyhydric alcohol.
  9. The cellulosic fiber of claim 1, wherein the phase change material includes one of a polyethylene glycol, a polyethylene oxide, a polytetramethylene glycol, and a polyester.
  10. The cellulosic fiber of claim 1, wherein the cellulosic fiber has a moisture absorbency in the range of 6 percent to 15 percent.

**40**

- 5 11. The cellulosic fiber of claim 1, wherein the cellulosic fiber is from 0.1 decitex to 60 decitex.
12. A fabric comprising:  
a plurality of cellulosic fibers blended together, the plurality of cellulosic fibers including a cellulosic fiber having enhanced reversible thermal properties and including:  
a fiber body including an elongated member, the elongated member including a cellulosic material and a temperature regulating material dispersed within the cellulosic material, the temperature regulating material including a phase change material having a transition temperature in the range of 0° C. to 50° C.  
wherein the cellulosic fiber is a first cellulosic fiber, the temperature regulating material is a first temperature regulating material, and the plurality of cellulosic fibers include a second cellulosic fiber having enhanced reversible thermal properties and including a second temperature regulating material.
- 15 13. The fabric of claim 12, wherein the first temperature regulating material and the second temperature regulating material are different.

\* \* \* \* \*